



US008450425B2

(12) **United States Patent**  
**Okabe et al.**

(10) **Patent No.:** **US 8,450,425 B2**  
(b5) **Date of Patent:** **\*May 28, 2013**

(54) **GOLF BALL**

(75) Inventors: **Satoko Okabe**, Kobe (JP); **Takahiro Shigemitsu**, Kobe (JP); **Kazuhiko Isogawa**, Kobe (JP); **Tsutomu Hirau**, Kobe (JP)

(73) Assignee: **SRI Sports Limited**, Kobe (JP)

(\*) Notice: Subject to any disclaimer, the term of this patent is extended or adjusted under 35 U.S.C. 154(b) by 719 days.  
This patent is subject to a terminal disclaimer.

(21) Appl. No.: **12/560,190**

(22) Filed: **Sep. 15, 2009**

(65) **Prior Publication Data**

US 2010/0069173 A1 Mar. 18, 2010

(30) **Foreign Application Priority Data**

Sep. 16, 2008 (JP) ..... 2008-237037  
Oct. 20, 2008 (JP) ..... 2008-269361  
Aug. 24, 2009 (JP) ..... 2009-193330

(51) **Int. Cl.**

**A63B 37/12** (2006.01)  
**A63B 37/00** (2006.01)  
**C08L 33/02** (2006.01)

(52) **U.S. Cl.**

USPC ..... **525/221**; 525/196; 525/201; 473/373;  
473/374; 473/378; 473/385

(58) **Field of Classification Search**

None

See application file for complete search history.

(56) **References Cited**

## U.S. PATENT DOCUMENTS

3,819,768 A 6/1974 Molitor et al.  
4,526,375 A 7/1985 Nakade  
5,292,794 A \* 3/1994 Maginnis ..... 524/556  
5,298,571 A \* 3/1994 Statz et al. ..... 525/330.2  
6,089,847 A 7/2000 Inoue et al.  
6,190,597 B1 2/2001 Inoue et al.  
6,235,230 B1 5/2001 Puniello  
6,238,194 B1 5/2001 Inoue et al.  
6,838,501 B2 1/2005 Takesue et al.  
6,962,951 B1 11/2005 Takesue et al.  
7,211,610 B2 5/2007 Takesue et al.  
2002/0037968 A1 \* 3/2002 Chen ..... 525/194  
2002/0099120 A1 7/2002 Takesue et al.  
2004/0132552 A1 7/2004 Chen  
2005/0256269 A1 11/2005 Takesue et al.  
2005/0261424 A1 \* 11/2005 Snell et al. ..... 525/7  
2006/0014898 A1 1/2006 Kim  
2006/0270491 A1 \* 11/2006 Jordan et al. ..... 473/371  
2006/0293121 A1 12/2006 Egashira et al.

2008/0220904 A1 9/2008 Sullivan et al.  
2008/0227569 A1 9/2008 Egashira et al.  
2010/0069173 A1 3/2010 Okabe et al.  
2010/0069177 A1 \* 3/2010 Okabe ..... 473/385  
2010/0075777 A1 \* 3/2010 Shigemitsu et al. ..... 473/372  
2010/0167846 A1 \* 7/2010 Hirau et al. ..... 473/378  
2010/0298066 A1 11/2010 Kim

## FOREIGN PATENT DOCUMENTS

JP 2-88087 A 3/1990  
JP 9-313646 A 12/1997  
JP 11-76466 A 3/1999  
JP 11-151323 A 6/1999  
JP 11-164914 A 6/1999  
JP 2001-120686 A 5/2001  
JP 2002-219195 A 8/2002  
JP 2005-230212 A 9/2005  
JP 3751824 A 12/2005  
JP 2006-500995 T 1/2006  
JP 2006-28517 A 2/2006  
JP 2007-622 A 1/2007

## OTHER PUBLICATIONS

Honeywell Product Literature for AClyn 295P; no date.\*  
Honeywell Product Literature for AClyn 201A; no date.\*  
English translation of Japanese Office Action dated Mar. 22, 2011, for Application No. 2008-269361.

English translation of the Japanese Office Action dated Apr. 19, 2011, for Application No. 2008-335603.

U.S. Office Action dated May 31, 2012, for U.S. Appl. No. 12/557,785.

U.S. Office Action dated May 31, 2012, for U.S. Appl. No. 12/554,155.

U.S. Office Action dated Sep. 14, 2012, for U.S. Appl. No. 12/627,460.

\* cited by examiner

Primary Examiner — David Buttner

(74) Attorney, Agent, or Firm — Birch, Stewart, Kolasch & Birch, LLP

(57) **ABSTRACT**

An object of the present invention is to provide a golf ball excellent in fluidity, adhesion of the paint film, and repulsion. Another object of the present invention is to provide a golf ball which is excellent in durability and low-temperature durability. The present invention provides a golf ball comprising: a core and a cover covering the core, wherein the cover is formed from a cover composition that contains as a resin component, (a) a specific high melt viscosity ionomer resin being neutralized with at least two metal ions, and (b) a low melt viscosity ionomer resin being neutralized with at least two metal ions, in a ratio of (a) the high melt viscosity ionomer resin/(b) the low melt viscosity ionomer resin being 55 mass % to 99 mass %/45 mass % to 1 mass %, wherein at least one of metal ions neutralizing carboxyl groups of (a) the high melt viscosity ionomer resin and/or (b) the low melt viscosity ionomer resin is a divalent metal ion and a content of the divalent metal ion per 100 g of the resin component is at least 0.020 mole.

2

Fig. 1



Fig.2



Fig.3

**1**  
**GOLF BALL**

**FIELD OF THE INVENTION**

The present invention relates to a golf ball, in particular, relates to a technology for molding a cover and improving the cover property.

**DESCRIPTION OF THE RELATED ART**

Ionomer resins are used as a cover material for the golf ball, because of its excellent durability and repulsion performance. However, the heat stability and moldability are also necessary to prepare golf balls using ionomer resins. Further, the obtained golf balls are required to show the excellent shot feeling, controllability, repulsion performance and durability.

From these aspects, various improvements have been proposed for golf balls using ionomer resins as a cover material. Japanese Patent Publication No. 2002-219195 A discloses a golf ball material that provides a high performance golf ball having an excellent repulsion as well as a good thermal stability, fluidity, and moldability. The golf ball material comprises a mixture which is composed of essential components:

100 pars by weight of a resinous component consisting of a base resin and (e) a non-ionomer thermoplastic elastomer, the base resin and the elastomer being blended in a weight ratio of 100:0 to 50:50;

(c) 5 to 80 parts by weight of a fatty acid and/or fatty acid derivative having a molecular weight of 280 to 1,500; and

(d) 0.1 to 10 parts by weight of a basic inorganic metal compound capable of neutralizing acidic groups left unneutralized in the base resin and component (c), wherein the base resin has (a) an olefin-unsaturated carboxylic acid binary random copolymer and/or a metal ion-neutralized olefin-unsaturated carboxylic acid binary random copolymer, blended with (b) an olefin-unsaturated carboxylic acid-unsaturated carboxylate ternary random copolymer and/or a metal ion neutralized olefin-unsaturated carboxylic acid-unsaturated carboxylate ternary random copolymer, in a weight ratio of 100:0 to 25:75.

Japanese Patent Publication No. 2001-120686 A discloses a golf ball material containing a highly neutralized ionomer resin that provides a high performance golf ball having an excellent repulsion as well as good thermal stability, fluidity, and moldability. The golf ball material comprises a heated mixture having a melt index of 1.0 dg/min or more which is composed of:

100 parts by weight of (a) an olefin-unsaturated carboxylic acid random copolymer and/or an olefin-unsaturated carboxylic acid-unsaturated carboxylate random copolymer,

(b) 5 to 80 parts by weight of a fatty acid or a derivative thereof having a molecular weight of 280 or more, and

(c) 0.1 to 10 parts by weight of a basic inorganic metal compound capable of neutralizing acidic groups in components (a) and (b).

Japanese Patent Publication No. 2006-500995 T discloses a golf ball which has an improved softness and scuff resistance while maintaining the durability and flight distance. The golf ball employs a blend of ionomer resins that have a different molecular weight each other, that is, a blend of a high molecular weight ternary ionomer resin (molecular weight about 80,000 to 500,000) and a low molecular weight binary ionomer resin (molecular weight about 2,000 to 30,000).

**SUMMARY OF THE INVENTION**

In order to enhance the repulsion of the golf ball, there is an approach of making the cover thin. However, the ionomer

**2**

resin must have a high fluidity in order to make the thin cover. As a technology of improving the fluidity of the ionomer resin while maintaining the repulsion performance, it is known that a low molecular weight material such as a fatty acid is added to the ionomer resin having a high degree of neutralization. However, the addition of the low molecular weight material such as a fatty acid causes smoke generation during the molding. Further, the low molecular weight material component tends to bleed out of a surface of the golf ball body. As a result, the adhesion of the paint film is lowered when applying a paint to the surface of the golf ball.

The present invention has been achieved in view of the above circumstances. An object of the present invention is to provide a golf ball excellent in the fluidity, adhesion of the paint film, and repulsion. Another object of the present invention is to provide a golf ball which is excellent in the durability and low-temperature durability.

Yet another object of the present invention is to provide a golf ball exhibiting a good adhesion of the paint film and the low-temperature durability as well as great flight distance and good shot feeling on the shots. Yet another object of the present invention is to provide a golf ball excellent in good direction stability on the shots.

The present invention provides a golf ball comprising:  
25 a core and a cover covering the core,  
wherein the cover is formed from a cover composition that contains as a resin component,

(a) a high melt viscosity ionomer resin having a melt viscosity (190° C.) ranging from 500 Pa·s to 100,000 Pa·s measured by a flow tester (hereinafter, simply referred to as "(a) the high melt viscosity ionomer resin" occasionally), and

(b) a low melt viscosity ionomer resin having a melt viscosity (190° C.) ranging from 1 Pa·s to 10 Pa·s measured by a brookfield viscometer and a melt flow rate (190° C. \*2.16 kg) 35 ranging from 100 g/10 min to 2,000 g/10 min (hereinafter, simply referred to as "(b) the low melt viscosity ionomer resin" occasionally),

in a ratio of (a) the high melt viscosity ionomer resin/(b) the low melt viscosity ionomer resin being 55 mass % to 99 mass %/45 mass % to 1 mass %, wherein at least one of metal ions neutralizing carboxyl groups of (a) the high melt viscosity ionomer resin and/or (b) the low melt viscosity ionomer resin is a divalent metal ion and the content of the divalent metal ion per 100 g of the resin component is at least 0.020 mole.

45 The present invention further provides a golf ball comprising:  
The present invention further provides a golf ball comprising:

a core and a cover covering the core,  
wherein the cover is formed from a cover composition that contains as a resin component,

(a) a high melt viscosity ionomer resin having a melt viscosity (190° C.) ranging from 500 Pa·s to 100,000 Pa·s measured by a flow tester and consisting of one prepared by neutralizing at least a part of carboxyl groups in a binary copolymer composed of ethylene and  $\alpha,\beta$ -unsaturated carboxylic acid having 3 to 8 carbon atoms with a metal ion, one prepared by neutralizing at least a part of carboxyl groups in a ternary copolymer composed of ethylene,  $\alpha,\beta$ -unsaturated carboxylic acid having 3 to 8 carbon atoms and  $\alpha,\beta$ -unsaturated carboxylate acid ester with a metal ion, or a mixture thereof, and

(b) a low melt viscosity ionomer resin having a melt viscosity (190° C.) ranging from 1 Pa·s to 10 Pa·s measured by a brookfield viscometer and a melt flow rate (190° C. \*2.16 kg) ranging from 100 g/10 min to 2,000 g/10 min, and consisting of one prepared by neutralizing at least a part of carboxyl groups in a binary copolymer composed of ethylene and  $\alpha,\beta$ -unsaturated carboxylic acid having 3 to 8 carbon atoms

with a metal ion, one prepared by neutralizing at least a part of carboxyl groups in a ternary copolymer composed of ethylene,  $\alpha,\beta$ -unsaturated carboxylic acid having 3 to 8 carbon atoms and  $\alpha,\beta$ -unsaturated carboxylic acid ester with a metal ion, or a mixture thereof,

in a ratio of (a) the high melt viscosity ionomer resin / (b) the low melt viscosity ionomer resin being 55 mass % to 99 mass %/45 mass % to 1 mass %, wherein at least one of metal ions neutralizing carboxyl groups of (a) the high melt viscosity ionomer resin and/or (b) the low melt viscosity ionomer resin is a divalent metal ion and a content of the divalent metal ion per 100 g of the resin component is at least 0.020 mole.

The present invention yet further provides a golf ball comprising:

a core consisting of at least one layer, an intermediate layer covering the core, and a cover covering the intermediate layer and having a thickness from 0.3 mm to 1.0 mm, wherein the cover is formed from a cover composition that contains as a resin component,

(a) a high melt viscosity ionomer resin having a melt viscosity (190° C.) ranging from 500 Pa·s to 100,000 Pa·s measured by a flow tester and consisting of one prepared by neutralizing at least a part of carboxyl groups in a binary copolymer composed of ethylene and  $\alpha,\beta$ -unsaturated carboxylic acid having 3 to 8 carbon atoms with a metal ion, one prepared by neutralizing at least a part of carboxyl groups in a ternary copolymer composed of ethylene,  $\alpha,\beta$ -unsaturated carboxylic acid having 3 to 8 carbon atoms and  $\alpha,\beta$ -unsaturated carboxylic acid ester with a metal ion, or a mixture thereof, and

(b) a low melt viscosity ionomer resin having a melt viscosity (190° C.) ranging from 1 Pa·s to 10 Pa·s measured by a brookfield viscometer and a melt flow rate (190° C. \*2.16 kg) ranging from 100 g/10 min to 2,000 g/10 min, and consisting of one prepared by neutralizing at least a part of carboxyl groups in a binary copolymer composed of ethylene and  $\alpha,\beta$ -unsaturated carboxylic acid having 3 to 8 carbon atoms with a metal ion, one prepared by neutralizing at least a part of carboxyl groups in a ternary copolymer composed of ethylene,  $\alpha,\beta$ -unsaturated carboxylic acid having 3 to 8 carbon atoms and  $\alpha,\beta$ -unsaturated carboxylic acid ester with a metal ion, or a mixture thereof,

in a ratio of (a) the high melt viscosity ionomer resin/(b) the low melt viscosity ionomer resin being 55 mass % to 99 mass %/45 mass % to 1 mass %,

wherein at least one of the metal ions neutralizing carboxyl groups of (a) the high melt viscosity ionomer resin and/or (b) the low melt viscosity ionomer resin is a divalent metal ion and a content of the divalent metal ion per 100 g of the resin component is at least 0.020 mole, and

wherein an intermediate layer composition forming the intermediate layer has a slab hardness from 35 to 55 in Shore D hardness.

In the present invention, since (a) the high melt viscosity ionomer resin component providing a high repulsion are blended as a main component with (b) the low melt viscosity ionomer resin which is a component for improving the fluidity, the cover composition exhibits a good fluidity and provides a golf ball having a high repulsion. Further, since (b) the low melt viscosity ionomer resin has a similar structure to (a) the high melt viscosity ionomer resin, the compatibility thereof is high. Thus, the bleed out of (b) the low melt viscosity ionomer resin from the surface of the golf ball body is suppressed. As a result, the golf balls excellent in the repulsion, fluidity, and the adhesion of the paint film are obtained. Further, the durability and the low-temperature durability of

the obtained golf ball are remarkably improved by employing a divalent metal ion as at least one metal ion neutralizing the carboxyl groups of (a) the high melt viscosity ionomer resin and/or (b) the low melt viscosity ionomer resin and making the content of the divalent metal ion at least 0.020 mole. Further, in a preferable embodiment, the lower spin on the driver shot is achieved by optimizing the hardness of the intermediate layer and employing the thin cover, which improves flight distance and direction stability and the shot 10 feeling is also improved by optimizing the hardness of the intermediate layer.

The present invention provides the golf ball excellent in the fluidity, the adhesion of the paint film, and the repulsion. Further, the present invention provides the golf ball excellent 15 in the durability and low-temperature durability.

The present invention also provides a golf ball exhibiting a good adhesion of the paint film and the low-temperature durability as well as great flight distance and good shot feeling on the shots. The present invention further provides a golf 20 ball excellent in good direction stability on the shots.

#### BRIEF DESCRIPTION OF THE DRAWINGS

FIG. 1 is an expanded sectional view of the dimples formed 25 on the surface of the golf ball body;

FIG. 2 is a top plan view of the dimple pattern formed on the surface of the golf ball; and

FIG. 3 is a front view of the dimple pattern formed on the 30 surface of the golf ball.

#### DESCRIPTION OF THE PREFERRED EMBODIMENT

The present invention provides a golf ball comprising: 35 a core and a cover covering the core, wherein the cover is formed from a cover composition that contains as a resin component,

(a) a high melt viscosity ionomer resin having a melt viscosity (190° C.) ranging from 500 Pa·s to 100,000 Pa·s measured by a flow tester, and

(b) a low melt viscosity ionomer resin having a melt viscosity (190° C.) ranging from 1 Pa·s to 10 Pa·s measured by a brookfield viscometer and a melt flow rate (190° C. \*2.16 kg) ranging from 100 g/10 min to 2,000 g/10 min,

in a ratio of (a) the high melt viscosity ionomer resin/(b) the low melt viscosity ionomer resin being 55 mass % to 99 mass %/45 mass % to 1 mass %, wherein at least one of metal ions neutralizing carboxyl groups of (a) the high melt viscosity ionomer resin and/or (b) the low melt viscosity ionomer resin is a divalent metal ion and a content of the divalent metal ion per 100 g of the resin component is at least 0.020 mole.

First, "(a) the high melt viscosity ionomer resin" contained in the cover composition will be explained.

(a) The high melt viscosity ionomer resin preferably contains one prepared by neutralizing at least a part of carboxyl groups in a binary copolymer composed of ethylene and  $\alpha,\beta$ -unsaturated carboxylic acid having 3 to 8 carbon atoms with a metal ion, one prepared by neutralizing at least a part of carboxyl groups in a ternary copolymer composed of ethylene,  $\alpha,\beta$ -unsaturated carboxylic acid having 3 to 8 carbon atoms, and  $\alpha,\beta$ -unsaturated carboxylic acid ester with a metal ion, or a mixture thereof.

Examples of the  $\alpha,\beta$ -unsaturated carboxylic acid having 3 to 8 carbon atoms are; acrylic acid, methacrylic acid, fumaric acid, maleic acid and crotonic acid. Among these, acrylic acid and methacrylic acid are particularly preferred. Examples of the  $\alpha,\beta$ -unsaturated carboxylic acid ester include methyl

ester, ethyl ester, propyl ester, n-butyl ester, isobutyl ester of acrylic acid, methacrylic acid, fumaric acid, and maleic acid. In particular, acrylic acid ester and methacrylic acid ester are preferable.

Examples of the metal ion for neutralizing at least a part of carboxyl groups of the binary copolymer composed of ethylene and  $\alpha,\beta$ -unsaturated carboxylic acid having 3 to 8 carbon atoms, and the ternary copolymer composed of ethylene,  $\alpha,\beta$ -unsaturated carboxylic acid having 3 to 8 carbon atoms, and  $\alpha,\beta$ -unsaturated carboxylic acid ester include: monovalent alkali metal ions such as sodium, potassium, lithium, and the like; divalent metal ions such as magnesium, calcium, zinc, barium, cadmium, and the like; trivalent metal ions such as aluminum and the like; and other metal ions such as tin, zirconium, and the like. Among them, zinc is preferable. The use of the divalent metal ion improves the durability and the low-temperature durability of the resultant golf ball.

(a) The high melt viscosity ionomer resin preferably contains one prepared by neutralizing at least a part of carboxyl groups in a binary copolymer composed of ethylene and (meth)acrylic acid with a metal ion, one prepared by neutralizing at least a part of carboxyl groups in a ternary copolymer composed of ethylene, (meth)acrylic acid, and (meth)acrylic acid ester with a metal ion, or a mixture thereof.

(a) The high melt viscosity ionomer resin more preferably contains an ionomer resin obtained by mixing (a-1) one prepared by neutralizing at least a part of carboxyl groups in a binary copolymer composed of ethylene and (meth)acrylic acid with a monovalent metal ion, and/or one prepared by neutralizing at least a part of carboxyl groups in a ternary copolymer composed of ethylene, (meth)acrylic acid, and (meth)acrylic acid ester with a monovalent metal ion, and (a-2) one prepared by neutralizing at least a part of carboxyl groups in a binary copolymer composed of ethylene and (meth)acrylic acid with a divalent metal ion, and/or one prepared by neutralizing at least a part of carboxyl groups in a ternary copolymer composed of ethylene, (meth)acrylic acid, and (meth)acrylic acid ester with a divalent metal ion.

The use of the above described mixture of the ionomer resins enhances the repulsion resilience of the cover composition. Herein, (meth)acrylic acid means acrylic acid or methacrylic acid. Examples of the monovalent metal ions are sodium, potassium, lithium, rubidium, cesium, and francium and examples of the divalent metal ions are magnesium, calcium, zinc, beryllium, strontium, barium, and radium. In this case, the blending ratio (a-1)/(a-2) is preferably 20 mass % to 80 mass % / 80 mass % to 20 mass %, more preferably 25 mass % to 77 mass % / 75 mass % to 23 mass %, even more preferably 30 mass % to 75 mass % / 70 mass % to 25 mass %.

The content of  $\alpha,\beta$ -unsaturated carboxylic acid having 3 to 8 carbon atoms in (a) the high melt viscosity ionomer resin is preferably 2 mass % or more, more preferably 3 mass % or more, and is preferably 30 mass % or less, more preferably 25 mass % or less.

The degree of neutralization of the carboxyl groups of the (a) the high melt viscosity ionomer resin is preferably 10 mole % or more, more preferably 15 mole % or more, and is preferably 90 mole % or less, more preferably 85 mole % or less. If the degree of the neutralization is 10 mole % or more, the repulsion and durability of the golf ball improves, while if the degree of the neutralization is 90 mole % or less, the fluidity of the cover composition improves (good moldability). The degree of neutralization of the carboxyl groups of the (a) the high melt viscosity ionomer resin can be calculated by the following mathematical expression.

Degree of neutralization (mole %) of (a) the high melt viscosity ionomer resin=(the number of moles of neutralized

carboxyl groups of the high melt viscosity ionomer resin/the number of moles of all carboxyl groups contained in the high melt viscosity ionomer resin)×100

The melt viscosity (190° C.) of (a) the high melt viscosity ionomer resin measured by a flow tester is 500 Pa·s or more, preferably 1,000 Pa·s or more, more preferably 1,500 Pa·s or more and is 100,000 Pa·s or less, preferably 95,000 Pa·s or less, more preferably 92,000 Pa·s or less. If the melt viscosity is 500 Pa·s or more, the durability of the resultant golf ball is improved, and while if the melt viscosity is 100,000 Pa·s or less, the moldability of the cover composition is improved.

Specific examples which can be used for the (a) the high melt viscosity ionomer resin include trade name "Himilan (registered trademark) (e.g. Himilan 1555 (Na), Himilan 1605 (Na), Himilan 1706 (Zn), Himilan 1707 (Na), Himilan AM7311 (Mg), Himilan AM7329 (Zn), Himilan 1856 (Na), Himilan 1855 (Zn), and the like)" commercially available from Du Pont-Mitsui Polymers Co., Ltd.

Further, ionomer resins commercially available from E.I. du Pont de Nemours and Company include trade name "Surlyn (registered trademark) (e.g. Surlyn 8945 (Na), Surlyn 9945 (Zn), Surlyn 8140 (Na), Surlyn 8150 (Na), Surlyn 9120 (Zn), Surlyn 9150 (Zn), Surlyn 6910 (Mg), Surlyn 6120 (Mg), Surlyn 7930 (Li), Surlyn 7940 (Li), Surlyn AD8546 (Li); Surlyn 6320 (Mg), Surlyn 8120 (Na), Surlyn 8320 (Na), Surlyn 9320 (Zn), Surlyn 9320W (Zn) as a ternary copolymerized ionomer; and the like)", "HPF 1000 (Mg), HPF 2000 (Mg)", and the like.

Further, ionomer resins commercially available from ExxonMobil Chemical Corporation include trade name "Iotek (registered trademark) (e.g. Iotek 8000 (Na), Iotek 8030 (Na), Iotek 7010 (Zn), Iotek 7030 (Zn), and the like)". Examples of a ternary copolymerized ionomer are "Iotek 7510 (Zn), Iotek 7520 (Zn)" and the like.

It is noted that Na, Zn, Li, and Mg described in the parentheses after the trade names indicate metal types of neutralizing metal ions.

Next, "(b) the low melt viscosity ionomer resin" used in the present invention will be explained.

(b) The low melt viscosity ionomer resin preferably includes one prepared by neutralizing at least a part of carboxyl groups of the binary copolymer composed of ethylene and  $\alpha,\beta$ -unsaturated carboxylic acid having 3 to 8 carbon atoms with a metal ion, one prepared by neutralizing at least a part of carboxyl groups of the ternary copolymer composed of ethylene,  $\alpha,\beta$ -unsaturated carboxylic acid having 3 to 8 carbon atoms,  $\alpha,\beta$ -unsaturated carboxylic acid ester with a metal ion, or a mixture thereof. As the  $\alpha,\beta$ -unsaturated carboxylic acid having 3 to 8 carbon atoms, the same  $\alpha,\beta$ -unsaturated carboxylic acid having 3 to 8 carbon atoms constituting "(a) the high melt viscosity ionomer resin" can be exemplified.

Examples of a metal ion used to neutralize a part of carboxyl group of the binary copolymer composed of ethylene and  $\alpha,\beta$ -unsaturated carboxylic acid having 3 to 8 carbon atoms, and the ternary copolymer composed of ethylene,  $\alpha,\beta$ -unsaturated carboxylic acid having 3 to 8 carbon atoms,  $\alpha,\beta$ -unsaturated carboxylic acid ester include: monovalent metal ions such as sodium, potassium, lithium, and the like; divalent metal ions such as magnesium, calcium, zinc, barium, cadmium, and the like; trivalent metal ions such as aluminum and the like; and other metal ions such as tin, zirconium, and the like. These metal ions may be used solely or in combination of two or more thereof. Among these metal ions, (b) the low melt viscosity ionomer resin is preferably neutralized with the divalent metal ion such as magnesium, calcium, zinc, barium, cadmium, and the like.

The melt viscosity (190° C.) of (b) the low melt viscosity ionomer resin measured by a brookfield viscometer is preferably 1 Pa·s or more, more preferably 2 Pa·s or more, even more preferably 3 Pa·s or more, and is preferably 10 Pa·s or less, more preferably 9 Pa·s or less, even more preferably 8 Pa·s or less. If the melt viscosity of (b) the low melt viscosity ionomer resin is 1 Pa·s or more, the compatibility with (a) component becomes high and thus the durability of the resultant golf ball improves. While if the melt viscosity of (b) the low melt viscosity ionomer resin is 10 Pa·s or less, the improving effect of the fluidity of the cover composition becomes large.

The melt flow rate (190° C., 2.16 kg) of (b) the low melt viscosity ionomer resin is preferably 100 g/10 min or more, more preferably 150 g/10 min or more, and even more preferably 200 g/10 min or more, and is preferably 2,000 g/10 min or less, more preferably 1,900 g/10 min or less, and even more preferably 1,800 g/10 min or less. If the melt flow rate of (b) the low melt viscosity ionomer resin is 100 g/10 min or more, the improved effect of the fluidity of the cover composition is large, while if the melt flow rate is 2,000 g/10 min or less, the compatibility with (a) component becomes high and the durability of the resultant golf ball improves.

The content of  $\alpha,\beta$ -unsaturated carboxylic acid having 3 to 8 carbon atoms in (b) the low melt viscosity ionomer resin is preferably 2 mass % or more, more preferably 3 mass % or more, and is preferably 30 mass % or less, more preferably 20 mass % or less.

The degree of neutralization of the carboxyl groups of (b) the low melt viscosity ionomer resin is preferably 10 mole % or more, more preferably 15 mole % or more, even more preferably 20 mole % or more, and even more preferably 100 mole %.

The degree of neutralization of the carboxyl groups of (b) the low melt viscosity ionomer resin can be calculated by the following mathematical expression.

Degree of neutralization (mol %) of (b) the low melt viscosity ionomer resin = (the number of moles of carboxyl groups neutralized of the low melt viscosity ionomer resin/the total number of moles of carboxyl groups contained in the low melt viscosity ionomer resin)  $\times 100$

Specific examples of (b) the low melt viscosity ionomer resin are "Aclyn (registered trade name) 201 (Ca)," "Aclyn246 (Mg)," and "Aclyn295 (Zn)" available from Honeywell Inc.

The blending ratio of (a) the high melt viscosity ionomer resin/(b) the low melt viscosity ionomer resin contained in the cover composition is preferably 55 mass % to 99 mass %/45 mass % to 1 mass %. If the blending ratio falls within the above range, since the fluidity of the cover composition improves, it is possible to produce the thin cover. As a result, the repulsion and the durability of the resultant golf ball are improved. The blending ratio of (a) the high melt viscosity ionomer resin/(b) the low melt viscosity ionomer resin is preferably 58 mass % to 90 mass %/42 mass % to 10 mass %, more preferably 60 mass % to 85 mass %/40 mass % to 15 mass %.

In the cover composition of the present invention, at least one of metal ions neutralizing carboxyl groups of (a) the high melt viscosity ionomer resin and/or (b) the low melt viscosity ionomer resin is a divalent metal ion and the content of the divalent metal ion per 100 g of the resin component is at least 0.020 mole.

Examples of the divalent metal ions are Ca, Mg, and Zn. Among them, Zn is preferable. The use of Zn as the divalent metal ion improves the durability, especially the low-temperature durability.

The content of the divalent metal ion neutralizing the carboxyl groups means a total content of the divalent metal ion neutralizing the carboxyl groups of (a) the high melt viscosity ionomer resin and the divalent metal ion neutralizing the carboxyl groups of (b) the low melt viscosity ionomer resin, and is determined by the method later described.

The content of the divalent metal per 100 g of the resin component constituting the cover composition is preferably 0.020 mole or more, more preferably 0.025 mole or more, even more preferably 0.030 mole or more, even more preferably 0.035 mole or more. If the content of the divalent metal per 100 g of the resin component is 0.020 mole or more, the durability, especially the low-temperature durability is improved. The upper limit of the content of the divalent metal per 100 g of the resin component is preferably, but not limited to, 0.16 mole, more preferably 0.15 mole, even more preferably 0.12 mole. If the content of the divalent metal per 100 g of the resin component is too much, the fluidity of the cover composition and the repulsion of the resultant golf ball may be lowered.

In a preferable embodiment of the present invention, the resin component of the cover composition for the golf ball essentially consists of (a) the high melt viscosity ionomer resin and (b) the low melt viscosity ionomer resin. However, in another preferable embodiment, the cover composition may further contain (c) a nonionic thermoplastic resin having a melt viscosity measured by a flow tester ranging from 5 Pa·s to 3,000 Pa·s (hereinafter, simply referred to as "(c) the nonionic thermoplastic resin" occasionally) in addition to (a) the high melt viscosity ionomer resin and (b) the low melt viscosity ionomer resin. Herein, the term "nonionic" means that there is no ionic center where an acid component (preferably, carboxyl group) is neutralized.

In this case, the resin component preferably comprises each component in the content of (a) the high melt viscosity ionomer resin: 45 mass % to 70 mass %, (b) the low melt viscosity ionomer resin: 5 mass % to 25 mass %, and (c) the nonionic thermoplastic resin: 10 mass % to 40 mass %, even more preferably in the content of (a) the high melt viscosity ionomer resin: 50 mass % to 68 mass %, (b) the low melt viscosity ionomer resin: 6 mass % to 20 mass %, and (c) the nonionic thermoplastic resin: 11 mass % to 35 mass %.

Examples of (c) the nonionic thermoplastic resin that can be contained in the cover composition for the golf ball of the present invention are a thermoplastic polyamide elastomer having a commercial name of "Pebax (registered trademark) (e.g. "Pebax 2533")) commercially available from Arkema K. K.; an ethylene-methacrylic acid copolymer having a commercial name of "NUCREL (registered trademark) (e.g. NUCREL N1050H, NUCREL N2050H, NUCREL N1110H, NUCREL N0200H) or an ethylene-acrylic acid copolymer having a commercial name of "PRIMACOR (registered trademark)" 5990I" available from Du Pont-Mitsui Polymers Co., Ltd.; a thermoplastic polyester elastomer having a commercial name of "Hytrel (registered trademark) (e.g. "Hytrel 3548", "Hytrel 4047")) commercially available from Du Pont-Toray Co., Ltd.; a thermoplastic polystyrene elastomer having a commercial name of "Rabalon (registered trademark)" and a thermoplastic polyester elastomer having a commercial name of "Primalloy (registered trademark) (e.g. "Primalloy A1500")) commercially available from Mitsubishi Chemical Corporation; a polyurethane elastomer having a commercial name of "Elastollan (registered trademark) (e.g. "Elastollan ET880")) commercially available from BASF Japan Ltd.

The melt viscosity (190° C.) of (c) the nonionic thermoplastic resin measured by a flow tester is preferably 5 Pa·s or

more, more preferably 10 Pa·s or more, even more preferably 15 Pa·s or more, and is preferably 3,000 Pa·s or less, more preferably 2,800 Pa·s or less, even more preferably 2,500 Pa·s or less. If the melt viscosity (190° C.) of (c) the nonionic thermoplastic resin is 5 Pa·s or more, the durability of the resultant golf ball improves, while if the melt viscosity is 3,000 Pa·s or less, the moldability of the cover composition improves.

In the present invention, in addition to the aforementioned resin component, the cover composition may further contain a pigment component such as a white pigment (for example, titanium oxide), a blue pigment (for example, ultramarine blue), a red pigment, and the like, a specific gravity adjusting agent such as zinc oxide, calcium carbonate, barium sulfate, and the like, a dispersant, an antioxidant, an ultraviolet absorber, a light stabilizer, a fluorescent material or a fluorescent brightener and the like, as long as they do not impair the performance of the cover.

The amount of the white pigment (titanium oxide), with respect to 100 parts by mass of the resin component constituting the cover, is preferably 0.5 part by mass or more, more preferably 1 part by mass or more, and is preferably 10 parts by mass or less, more preferably 8 parts by mass or less. By causing the amount of the white pigment to be 0.5 parts by mass or more, it is possible to impart the opacity to the cover. If the amount of the white pigment is more than 10 parts by mass, there is the possibility that the durability of the resultant cover will deteriorate.

In the present invention, the melt flow rate (190° C., 2.16 kg) of the cover composition is preferably 10 g/10 min or more, more preferably 15 g/10 min or more, and even more preferably 20 g/10 min or more, and is preferably 100 g/10 min or less, more preferably 95 g/10 min or less, and even more preferably 90 g/10 min or less. If the melt flow rate of the cover composition is 10 g/10 min or more, the moldability of the cover composition is enhanced.

The cover composition preferably has a bending stiffness of 100 MPa or more, more preferably 110 MPa or more, even more preferably 120 MPa or more, and preferably has a bending stiffness of 450 MPa or less, more preferably 420 MPa or less, even more preferably 400 MPa or less. If the bending stiffness of the cover composition is 100 MPa or more, since the obtained golf ball has an outer-hard inner soft structure, the flight distance becomes great. On the other hand, if the bending stiffness is 450 MPa or less, the cover becomes appropriately soft and thus the shot feeling of the golf ball becomes good.

The cover composition preferably has a repulsion resilience of 40% or more, more preferably 41% or more, even more preferably 42% or more. If the repulsion resilience of the cover composition is 40% or more, the flight distance of the obtained golf ball becomes great. Herein, the bending stiffness and the repulsion resilience of the cover composition are measured by forming the cover composition into a sheet form. The method for the measurement is described later.

The cover composition preferably has a slab hardness of 40 or more, more preferably 45 or more, even more preferably 50 or more, and preferably has a slab hardness of 70 or less, more preferably 68 or less, even more preferably 65 or less in Shore D hardness. If the cover composition has a slab hardness of 40 or more, the stiffness of the resultant cover is enhanced, and thus the golf ball excellent in the repulsion (flight distance) is obtained. On the other hand, if the cover composition has a slab hardness of 70 or less, the durability is more enhanced. Herein, the slab hardness of the cover composition is a measured hardness of the cover composition that is molded into a sheet form by a measuring method described later.

An embodiment for molding a cover is not particularly limited, and includes an embodiment which comprises injection molding the cover composition directly onto the core, or an embodiment which comprises molding the cover composition into a hollow-shell, covering the core with a plurality of the hollow-shells and subjecting the core with a plurality of the hollow shells to the compression-molding (preferably an embodiment which comprises molding the cover composition into a half hollow-shell, covering the core with the two half hollow-shells, and subjecting the core with the two half hollow-shells to the compression-molding). In the case of directly injection molding the cover composition onto the core, it is preferred to use upper and lower molds for forming a cover having a spherical cavity and pimples, wherein a part of the pimple also serves as a retractable hold pin. When forming the cover by injection molding, the hold pin is protruded to hold the core, and the cover composition which has been heated and melted is charged and then cooled to obtain a cover. For example, the cover composition heated and melted at the temperature of 150° C. to 230° C. is charged into a mold held under the pressure of 980 KPa to 1,500 KPa for 0.1 to 1 second. After cooling for 15 to 60 seconds, the mold is opened and the golf ball with the cover molded is taken out from the mold.

When molding the cover in a compression molding method, molding of the half shell can be performed by either compression molding method or injection molding method, and the compression molding method is preferred. The compression-molding of the cover composition into half shell can be carried out, for example, under a pressure of 1 MPa or more and 20 MPa or less at a temperature of -20° C. or more and 70° C. or less relative to the flow beginning temperature of the cover composition. By performing the molding under the above conditions, a half shell having a uniform thickness can be formed. Examples of a method for molding the cover using half shells include compression molding by covering the core with two half shells. The compression molding of half shells into the cover can be carried out, for example, under a pressure of 0.5 MPa or more and 25 MPa or less at a temperature of -20° C. or more and 70° C. or less relative to the flow beginning temperature of the cover composition. By performing the molding under the above conditions, a cover for a golf ball having a uniform thickness can be formed.

The molding temperature means the highest temperature where the temperature at the surface of the concave portion of the lower mold reaches from closing through opening the molds. Further, the flow beginning temperature of the cover material can be measured in a pellet form with the following conditions by using a flow characteristics evaluation apparatus (Flow Tester CFT-500D, manufactured by Shimadzu Corporation).

Measuring conditions: Area size of a plunger: 1 cm<sup>2</sup>, Die length: 1 mm, Die diameter: 1 mm, Load: 588.399 N, Start temperature: 30° C., and Temperature increase rate: 3° C./min.

When molding a cover, the concave portions called "dimple" are usually formed on the surface. FIG. 1 is an expanded sectional view of a part of a golf ball 2. This figure shows a cross-section which includes the deepest part De of a dimple 10 and the center of the golf ball 2. The up and down direction in FIG. 1 is the depth direction of the dimple 10. The depth direction is the direction from the gravity center of the area of the dimple 10 to the center of the golf ball 2. A chain double-dashed line 14 in FIG. 1 shows a virtual sphere. The surface of the virtual sphere 14 is the surface of the golf ball 2 in the case of assuming that there is no dimple 10. The dimple 10 is depressed in the virtual sphere 14. A land 12

## 11

corresponds to the virtual sphere 14. In FIG. 1, the distance between the tangent line T and the deepest point De is the depth of the dimple 10.

Two headed arrow Di in FIG. 1 shows the diameter of the dimple 10. The diameter Di is the distance from one contact point Ed to another contact point Ed when a common tangent line T is drawn in both sides of the dimple 10. The contact points Ed are edges of the dimple 10. The edges Ed define the outline of the dimple 10. The diameter Di is preferably 2.0 mm or more and 6.0 mm or less. If the diameter Di is less than the above range, the dimple effect is hardly obtained and if the diameter Di exceeds 6.0 mm, the intrinsic property of the golf ball 2, that is, it is substantially spherical, is lost. The volume of the dimple means the volume of the portion surrounded with the curved plane including the outline of the dimple 10 and the virtual sphere 14. The total volume of the dimples 10 is preferably 250 mm<sup>3</sup> or more and 400 mm<sup>3</sup> or less. If the total volume is less than 250 mm<sup>3</sup>, a hopping trajectory may be provided in some cases. If the total volume exceeds 400 mm<sup>3</sup>, a dropping trajectory may possibly be provided.

In FIG. 1, the distance between the tangent line T and the deepest point De is the depth of the dimple 10. The depth is preferably 0.05 mm or more and 0.60 mm or less. If the depth is less than 0.05 mm, a hopping trajectory may be provided in some cases. On the other hand, if the depth exceeds 0.60 mm, a dropping trajectory may possibly be provided. The total number of the dimples 10 is preferably 200 or more and 500 or less. If the total number is less than 200, the dimple effect is hardly obtained. On the other hand, if the total number exceeds 500, the dimple effect is hardly obtained because the size of the respective dimples 10 is small. The shape (shape in a plan view) of dimples 10 includes, for example, without limitation, a circle, polygonal shapes such as roughly triangular shape, roughly quadrangular shape, roughly pentagonal shape, and roughly hexagonal shape, another irregular shape. The shape of the dimples is employed solely or in combination at least two of them. After the cover is molded, the mold is opened and the golf ball body is taken out from the mold, and as necessary, the golf ball body is preferably subjected to surface treatments such as deburring, cleaning, and sandblast. If desired, a paint film or a mark may be formed.

The present invention may further include a coated golf ball that comprises a golf ball body consisting of a core and a cover covering the core and a paint film covering the golf ball body.

The resin component constituting the paint film includes, without limitation, an acrylic resin, an epoxy resin, a polyurethane resin, a polyester resin, a cellulose resin. Among them, the two part curing type polyurethane resin described later is preferably used. The use of the two part curing type polyurethane resin provides a paint film with a more excellent durability.

The two part curing type polyurethane resin is a polyurethane resin that is cured by reacting a base material and a curing agent. For example, the two part curing type polyurethane resin is obtained by curing the base material containing a polyol component with a polyisocyanate compound or a derivative thereof. The base material containing the polyol component preferably contains a urethane polyol, which is obtained by reacting the polyisocyanate compound with the polyol.

The paint film preferably has a thickness of, but not limited to, 5  $\mu\text{m}$  or larger, and more preferably 7  $\mu\text{m}$  or larger, and preferably has a thickness of 25  $\mu\text{m}$  or smaller, and more preferably 18  $\mu\text{m}$  or smaller. This is because if the thickness is smaller than 5  $\mu\text{m}$ , the paint film is easy to wear off due to continued use of the golf ball, and if the thickness is larger

## 12

than 25  $\mu\text{m}$ , the effect of the dimples is reduced, resulting in the low flying performance of the golf ball.

In the present invention, the thickness of the cover of the golf ball is preferably 3 mm or less, more preferably 2.5 mm or less, and even more preferably 2 mm or less, even more preferably 1.5 mm or less. This is because by causing the thickness of the cover to be 3 mm or less, the desirable repulsion and shot feeling are obtained. The thickness of the cover is preferably 0.1 mm or more, more preferably 0.2 mm or more, and even more preferably 0.3 mm or more. This is because if the thickness of the cover is less than 0.1 mm, it may become difficult to mold the cover. In addition, the durability and the abrasion resistance of the cover may deteriorate.

Next, the preferable core of the golf ball of the present invention is explained. The core of the golf ball of the present invention includes, for example, a single-layered core, a core consisting of a center and a single-layered intermediate layer covering the center, a core consisting of a center and multi-piece or multi-layer of intermediate layers covering the center. The core preferably has a spherical shape. If the core does not have a spherical shape, the cover does not have a uniform thickness. As a result, there exist some portions where the performance of the cover is lowered. On the other hand, the center generally has the spherical shape, but the center may be provided with a rib on the surface thereof so that the surface of the spherical center is divided by the ribs. For example, the surface of the spherical center is evenly divided by the ribs. In one embodiment, the ribs are preferably formed on the surface of the spherical center in an integrated manner, and in another embodiment, the ribs are formed as an intermediate layer on the surface of the spherical center.

The ribs are preferably formed along an equatorial line and meridians that evenly divide the surface of the spherical center, if the spherical center is assumed as the earth. For example, if the surface of the spherical center is evenly divided into 8, the ribs are formed along the equatorial line, any meridian as a standard, and meridians at the longitude 90 degrees east, longitude 90 degrees west, and the longitude 180 degrees east(west), assuming that the meridian as the standard is at longitude 0 degree. If the ribs are formed, the depressed portion divided by the ribs are preferably filled with a plurality of intermediate layers or with a single-layered intermediate layer that fills each of the depressed portions to make a core in the spherical shape. The shape of the ribs, without limitation, includes an arc or an almost arc (for example, a part of the arc is removed to obtain a flat surface at the cross or orthogonal portions thereof).

As the center or the core of the golf ball of the present invention, a conventionally known rubber composition (hereinafter simply referred to as "core rubber composition" occasionally) may be employed, and it can be molded by, for example, heat-pressing a rubber composition containing a base rubber, a crosslinking initiator, a co-crosslinking agent, and a filler.

As the base rubber, a natural rubber and/or a synthetic rubber may be used. Examples of the base rubber are a polybutadiene rubber, a natural rubber, a polyisoprene rubber, a styrene polybutadiene rubber, and ethylene-propylene-diene terpolymer (EPDM). Among them, typically preferred is the high cis-polybutadiene having cis-1,4-bond in a proportion of 40% or more, more preferably 70% or more, even more preferably 90% or more in view of its superior repulsion property.

The crosslinking initiator is blended to crosslink the base rubber component. As the crosslinking initiator, an organic peroxide is preferably used. Examples of the organic perox-

ide for use in the present invention are dicumyl peroxide, 1,1-bis(t-butylperoxy)-3,5-trimethylcyclohexane, 2,5-dimethyl-2,5-di(t-butylperoxy)hexane, and di-t-butyl peroxide. Among them, dicumyl peroxide is preferable. An amount of the crosslinking initiator to be blended in the rubber composition is preferably 0.2 part by mass or more, more preferably 0.3 part by mass or more, and is preferably 3 parts by mass or less, more preferably 2 parts by mass or less based on 100 parts by mass of the base rubber. If the amount is less than 0.2 part by mass, the core becomes too soft, and the repulsion tends to be lowered, and if the amount is more than 3 parts by mass, the amount of the co-crosslinking agent must be increased in order to obtain the appropriate hardness, which tends to cause the insufficient repulsion.

The co-crosslinking agent is not particularly limited as long as it serves to crosslink a rubber molecule by graft polymerization with a base rubber molecular chain; for example,  $\alpha, \beta$ -unsaturated carboxylic acid having 3 to 8 carbon atoms or a metal salt thereof, more preferably acrylic acid, methacrylic acid or a metal salt thereof may be used. As the metal constituting the metal salt, for example, zinc, magnesium, calcium, aluminum and sodium may be used, and among them, zinc is preferred because it provides high repulsion. The amount of the co-crosslinking agent to be used is preferably 10 parts or more, more preferably 20 parts or more, and is preferably 50 parts or less, more preferably 40 parts or less, based on 100 parts of the base rubber by mass. If the amount of the co-crosslinking agent to be used is less than 10 parts by mass, the amount of the crosslinking initiator must be increased to obtain an appropriate hardness, which tends to lower the repulsion. On the other hand, if the amount of the co-crosslinking agent to be used is more than 50 parts by mass, the core becomes too hard, so that the shot feeling may be lowered.

The filler contained in the core rubber composition is mainly blended as a specific gravity adjusting agent in order to adjust the specific gravity of the golf ball obtained as the final product in the range of 1.0 to 1.5, and may be blended as required. Examples of the filler include an inorganic filler such as zinc oxide, barium sulfate, calcium carbonate, magnesium oxide, tungsten powder, and molybdenum powder. The amount of the filler to be blended in the rubber composition is preferably 2 parts or more, more preferably 3 parts or more, and preferably 50 parts or less, more preferably 35 parts or less based on 100 parts of the base rubber by mass. If the amount of the filler to be blended is less than 2 parts by mass, it becomes difficult to adjust the weight, while if it is more than 50 parts by mass, the weight ratio of the rubber component becomes small and the repulsion tends to be lowered.

As the core rubber composition, an organic sulfur compound, an antioxidant or a peptizing agent may be blended appropriately in addition to the base rubber, the crosslinking initiator, the co-crosslinking agent and the filler.

As the organic sulfur compound, a diphenyl disulfide or a derivative thereof may be preferably used. Examples of the diphenyl disulfide or the derivative thereof include diphenyl disulfide, a mono-substituted diphenyl disulfide such as bis(4-chlorophenyl)disulfide, bis(3-chlorophenyl)disulfide, bis(4-bromophenyl) disulfide, bis(3-bromophenyl)disulfide, bis(4-fluorophenyl)disulfide, bis(4-iodophenyl)disulfide and bis(4-cyanophenyl)disulfide; a di-substituted diphenyl disulfide such as bis(2,5-dichlorophenyl)disulfide, bis(3,5-dichlorophenyl) disulfide, bis(2,6-dichlorophenyl)disulfide, bis(2,5-dibromophenyl)disulfide, bis(3,5-dibromophenyl)disulfide, bis(2-chloro-5-bromophenyl)disulfide, and bis(2-cyano-5-bromophenyl)disulfide; a tri-substituted diphenyl disulfide such as bis(2,4,6-trichlorophenyl)disulfide, and bis

(2-cyano-4-chloro-6-bromophenyl) disulfide; a tetra-substituted diphenyl disulfide such as bis(2,3,5,6-tetra chlorophenyl)disulfide; a penta-substituted diphenyl disulfide such as bis(2,3,4,5,6-pentachlorophenyl)disulfide and bis(2,3,4,5,6-pentabromophenyl) disulfide. These diphenyl disulfides or the derivative thereof can enhance repulsion by having some influence on the state of vulcanization of vulcanized rubber. Among them, diphenyl disulfide and bis(pentabromophenyl) disulfide are preferably used since a golf ball having particularly high repulsion can be obtained. The amount of the diphenyl disulfide or the derivative thereof to be blended is preferably 0.1 part by mass or more, more preferably 0.3 part by mass or more, and preferably 5.0 parts by mass or less, more preferably 3.0 parts by mass or less relative to 100 parts by mass of the base rubber.

The amount of the antioxidant to be blended is preferably 0.1 part or more and is preferably 1 part or less based on 100 parts of the base rubber by mass. Further, the amount of the peptizing agent is preferably 0.1 part or more and is preferably 5 parts or less based on 100 parts of the base rubber by mass.

The conditions for press-molding the core rubber composition should be determined appropriately depending on the rubber composition. The press-molding is preferably carried out for 10 to 60 minutes at the temperature of 130°C. to 200°C. under the pressure of 2.9 MPa to 11.8 MPa. For example, the press-molding is preferably carried out at the temperature from 130°C. to 180°C. for 10 to 40 minutes. Alternatively, the press-molding is preferably carried out in a two-step heating, for example, for 20 to 40 minutes at the temperature of 130°C. to 150°C., and continuously for 5 to 15 minutes at the temperature of 160°C. to 180°C.

The diameter of the core of the golf ball of the present invention is preferably 39.0 mm or more, more preferably 39.5 mm or more, and even more preferably 40.8 mm or more. If the diameter of the core is less than 39.0 mm, the cover becomes excessively thick and hence the repulsion of the golf ball may deteriorate. Further, the diameter of the core is preferably 42.2 mm or less, more preferably 42.0 mm or less, and even more preferably 41.8 mm or less. If the diameter of the core is more than 42.2 mm, the thickness of the cover becomes relatively thin, and hence a protection effect of the cover is not obtained sufficiently.

A compression deformation amount (shrinking deformation amount of the core along the compression direction) of the core when applying a load from 98 N as an initial load to 1275 N as a final load is preferably 2.50 mm or more, more preferably 2.60 mm or more, even more preferably 2.70 mm or more, and is preferably 3.20 mm or less, more preferably 3.10 mm or less, even more preferably 3.00 mm or less. If the compression deformation amount is less than 2.50 mm, the core becomes too hard, resulting in the poor shot feeling, while if the compression deformation amount is more than 3.20 mm, the core becomes too soft, resulting in the heavy shot feeling.

It is preferable that the core of the present invention has a larger surface hardness (Hs) than the center hardness (Ho). The hardness difference between the surface hardness (Hs) and the center hardness (Ho) of the core in the golf ball of the present invention is preferably 7 or larger, more preferably 10 or larger, even more preferably 13 or larger in Shore D hardness. If the surface hardness (Hs) is larger than the center hardness (Ho), the effect of lowering spin rate becomes large, thereby improving the flight distance of the golf ball. On the other hand, the hardness difference between the surface hardness (Hs) and the center hardness (Ho) of the core in the golf ball of the present invention is preferably 25 or less, more

## 15

preferably 20 or less, even more preferably 17 or less in Shore D hardness. If the hardness difference is too large, the durability of the golf ball may deteriorate. The hardness difference of the core is made by appropriately controlling the heating condition of the core or by employing a multi-layered core.

The center hardness (Ho) of the core is preferably 30 or larger, more preferably 33 or larger, and even more preferably 36 or larger in Shore D hardness. If the center hardness (Ho) is smaller than 30 in Shore D hardness, the core becomes so soft that the repulsion of the golf ball tends to be lower. The center hardness (Ho) of the core is preferably 50 or smaller, more preferably 47 or smaller, and even more preferably 43 or smaller in Shore D. If the center hardness (Ho) is 50 or smaller in Shore D hardness, the core does not become too hard, resulting in the good shot feeling. In the present invention, the center hardness (Ho) of the core is the hardness measured with the Shore D type spring hardness tester at the central point of a cut plane of a core which has been cut into two halves.

The surface hardness (Hs) of the core is preferably 44 or larger, more preferably 47 or larger, and even more preferably 50 or larger in Shore D hardness. If the surface hardness is 44 or more, the core does not become so soft and the good repulsion is obtained. The surface hardness of the core is preferably 60 or smaller, more preferably 57 or smaller, and even more preferably 55 or smaller in shore D hardness. If the surface hardness is 60 or less in Shore D hardness, the core does not become so hard and the good shot feeling is obtained.

In the case that the core consists of a center and a single layered intermediate layer covering the center, or that the core consists of a center and multi-piece of intermediate layers or multi-layer of intermediate layers covering the center, a material for the intermediate layer includes, for example, a thermoplastic resin such as a polyurethane resin, ionomer resin, nylon, and polyethylene, and a thermoplastic elastomer such as a polystyrene elastomer, polyolefin elastomer, polyurethane elastomer, polyester elastomer. Among them, the ionomer resin is preferable.

The intermediate layer of the golf ball of the present invention may contain a specific gravity adjusting agent such as barium sulfate and tungsten, an anti-oxidant, and a pigment in addition to the above resin component.

When the golf ball of the present invention has a diameter in a range from 40 mm to 45 mm, a compression deformation amount of the golf ball (an amount of compression of the golf ball in the compression direction thereof) when applying an initial load of 98 N to a final load of 1275 N to the golf ball is preferably 2.0 mm or more, more preferably 2.2 mm or more, and is preferably 4.0 mm or less, more preferably 3.5 mm or less. By causing the compression deformation amount to be 2.0 mm or more, the golf ball does not become too hard and the desirable shot feeling is obtained. By causing the compression deformation amount to be 4.0 mm or less, the repulsion is enhanced.

The golf ball of the present invention is not particularly limited on a structure thereof as long as the golf ball has a core and a cover. Examples of the golf ball of the present invention include a two-piece golf ball comprising a single-layered core, and a cover covering the core; a three-piece golf ball comprising a core consisting of a center and an intermediate layer covering the center, and a cover covering the core; a multi-piece golf ball comprising a core consisting of a center and a multi-piece or multi-layer of intermediate layers covering the center, and a cover covering the core; and a wound

## 16

golf ball comprising a wound core, and a cover covering the wound core. The present invention can be suitably applied to anyone of the above golf ball.

When preparing a wound golf ball in the present invention, 5 a wound core may be used as the core. In that case, for example, a wound core comprising a center formed by curing the above core rubber composition and a rubber thread layer which is formed by winding a rubber thread around the center in an elongated state can be used. In the present invention, the 10 rubber thread, which is conventionally used for winding around the center, can be adopted for winding around the center. The rubber thread, for example, is obtained by vulcanizing a rubber composition including a natural rubber, or a mixture of a natural rubber and a synthetic polyisoprene, a sulfur, a vulcanization auxiliary agent, a vulcanization accelerator, and an antioxidant. The rubber thread is wound around the center in elongation of about 10 times length to form the wound core.

20 In a preferable embodiment, the present invention is directed to a golf ball comprising:

a core consisting of at least one layer,  
an intermediate layer covering the core, and  
a cover covering the intermediate layer and having a thickness from 0.3 mm to 1.0 mm,

25 wherein the cover is formed from a cover composition that contains as a resin component,

(a) a high melt viscosity ionomer resin having a melt viscosity (190° C.) ranging from 500 Pa·s to 100,000 Pa·s measured by a flow tester and consisting of one prepared by neutralizing at least a part of carboxyl groups in a binary copolymer composed of ethylene and  $\alpha,\beta$ -unsaturated carboxylic acid having 3 to 8 carbon atoms with a metal ion, one prepared by neutralizing at least a part of carboxyl groups in 30 a ternary copolymer composed of ethylene,  $\alpha,\beta$ -unsaturated carboxylic acid having 3 to 8 carbon atoms and  $\alpha,\beta$ -unsaturated carboxylic acid ester with a metal ion, or a mixture thereof, and

(b) a low melt viscosity ionomer resin having a melt viscosity (190° C.) ranging from 1 Pa·s to 10 Pa·s measured by a brookfield viscometer and a melt flow rate (190° C. \*2.16 kg) ranging from 100 g/10 min to 2,000 g/10 min, and consisting of one prepared by neutralizing at least a part of carboxyl groups in a binary copolymer composed of ethylene and  $\alpha,\beta$ -unsaturated carboxylic acid having 3 to 8 carbon atoms with a metal ion, one prepared by neutralizing at least a part of carboxyl groups in a ternary copolymer composed of ethylene,  $\alpha,\beta$ -unsaturated carboxylic acid having 3 to 8 carbon atoms and  $\alpha,\beta$ -unsaturated carboxylic acid ester with a metal ion, or a mixture thereof,

40 in a ratio of (a) the high melt viscosity ionomer resin/(b) the low melt viscosity ionomer resin being 55 mass % to 99 mass %/45 mass % to 1 mass %,

45 wherein at least one of the metal ions neutralizing carboxyl groups of (a) the high melt viscosity ionomer resin and/or (b) the low melt viscosity ionomer resin is a divalent metal ion and the content of the divalent metal ion per 100 g of the resin component is at least 0.020 mole, and

50 wherein an intermediate layer composition forming the intermediate layer has a slab hardness from 35 to 55 in Shore D hardness.

In the preferable embodiment, the core of the golf ball of the present invention consists of at least one layer, and examples of the core are, without limitation, a single-layered core, a multi-layered core consisting of a center and a single-layered surrounding layer covering the center, and a multi-layered core consisting of a center and multi-piece or multi-

layer of surrounding layers covering the center. Among them, the single-layered core is preferable.

The surrounding layer composition forming the surrounding layer includes, for example, in addition to the rubber composition above described, and the ionomer resin exemplified as (a) the component, a thermoplastic polyamide elastomer having a commercial name of "Pebax (registered trademark) (e.g. "Pebax 2533")" commercially available from Arkema K. K.; a thermoplastic polyester elastomer having a commercial name of "Hytrel (registered trademark) (e.g. "Hytrel 3548", "Hytrel 4047")" commercially available from Du Pont-Toray Co., Ltd.; a polyurethane elastomer having a commercial name of "Elastollan (registered trademark) (e.g. "Elastollan XNY97A")" commercially available from BASF Japan Ltd; a thermoplastic polystyrene elastomer having a commercial name of "Rabalon (registered trademark) (e.g. "Rabalon T3221C")" commercially available from Mitsubishi Chemical Corporation. The surrounding layer composition may further contain a specific gravity adjusting agent such as barium sulfate and tungsten powder, an antioxidant, a pigment and the like.

The diameter of the core in the preferable embodiment is preferably 39.1 mm or more, more preferably 39.4 mm or more, and even more preferably 39.8 mm or more. If the diameter of the core is 39.1 mm or more, the core becomes large, resulting in the good repulsion. If the core becomes large, since the intermediate layer having a relatively high specific gravity is disposed in the outer part of the golf ball, the golf ball is designed to have an outer heavy inner light structure, which leads to the lower spin and the improved flight distance. On the other hand, the diameter of the core is preferably 40.7 mm or less, more preferably 40.5 mm or less, and even more preferably 40.1 mm or less. If the diameter of the core is 40.7 mm or less, the thickness of the intermediate layer and the cover does not become too thin, and hence the intermediate layer and the cover functions well.

Next, the intermediate layer covering the core will be explained.

The resin component of the intermediate layer composition forming the intermediate layer includes, for example, a thermoplastic polyamide elastomer having a commercial name of "Pebax (registered trademark) (e.g. "Pebax 2533")" commercially available from Arkema K. K.; a thermoplastic polyester elastomer having a commercial name of "Hytrel (registered trademark) (e.g. "Hytrel 3548", "Hytrel 4047")" commercially available from Du Pont-Toray Co., Ltd.; a polyurethane elastomer having a commercial name of "Elastollan (registered trademark) (e.g. "Elastollan XNY97A")" commercially available from BASF Japan Ltd; a thermoplastic polystyrene elastomer having a commercial name of "Rabalon (registered trademark) (e.g. "Rabalon T3221C")" commercially available from Mitsubishi Chemical Corporation, in addition to the ionomer resin. Examples of the ionomer resins are "Himalan (registered trademark) (e.g. Himalan AM7329 (Zn))" commercially available from Du Pont-Mitsui Polymers Co., Ltd, and "Surlyn (registered trademark) (e.g. Surlyn 8945 (Na))" commercially available from E.I. du Pont de Nemours and Company. These materials can be used solely or in combination at least two of them. Among them, in view of the repulsion, the intermediate layer composition preferably contains a mixture of the ionomer resin and the thermoplastic polystyrene elastomer as the resin component.

The intermediate layer composition may further contain a specific gravity adjusting agent, an antioxidant, a pigment and the like appropriately.

Examples of the specific gravity adjusting agent are zinc oxide, calcium carbonate, barium sulfate, tungsten, molyb-

denum and the like. The blending amount of the specific gravity adjusting agent is preferably 15 parts or more, more preferably 25 parts or more, even more preferably 30 parts or more, and is preferably 50 parts or less, more preferably 45 parts or less, even more preferably 40 parts or less, with respect to 100 parts of the resin component of the intermediate layer composition by mass. If the blending amount of the specific gravity adjusting agent is 15 parts or more by mass, it is easy to adjust the density of the intermediate layer composition, while if the blending amount is 50 parts or less by mass, it is possible to obtain the intermediate layer having a high density without impairing the durability of the golf ball.

The intermediate layer composition preferably has a slab hardness (Hm) of 35 or more, more preferably 40 or more, even more preferably 45 or more, and preferably has a slab hardness of 55 or less, more preferably 53 or less, even more preferably 50 or less in Shore D hardness. If the intermediate layer composition has a slab hardness (Hm) of 35 or more, the repulsion of the golf ball is enhanced. On the other hand, if the intermediate layer composition has a slab hardness of 55 or less, the shot feeling is enhanced. Herein, the slab hardness (Hm) of the intermediate layer composition is a measured hardness of the intermediate layer composition that is molded into a sheet form by a measuring method described later.

The intermediate layer composition preferably has a density of 1.10 g/cm<sup>3</sup> or more, more preferably 1.20 g/cm<sup>3</sup> or more, even more preferably 1.30 g/cm<sup>3</sup> or more. If the density of the intermediate layer composition is 1.10 g/cm<sup>3</sup> or more, the inertia moment of the golf ball can be high. On the other hand, the upper limit of the density of the intermediate layer is preferably, but not limited to, 2.00 g/cm<sup>3</sup>, more preferably 1.80 g/cm<sup>3</sup>, even more preferably 1.60 g/cm<sup>3</sup>. The intermediate layer having a high density is preferably disposed in the outer part of the golf ball as much as possible.

In this case, the core preferably has a density of 1.15 g/cm<sup>3</sup> or less, more preferably 1.13 g/cm<sup>3</sup> or less, even more preferably 1.10 g/cm<sup>3</sup> or less. If the core has the density of 1.15 g/cm<sup>3</sup> or less, the inertia moment of the golf ball can be high. On the other hand, the core preferably has a density of 0.96 g/cm<sup>3</sup> or more, more preferably 0.98 g/cm<sup>3</sup> or more, even more preferably 1.00 g/cm<sup>3</sup> or more. Further, it is noted that the density of the cover composition is preferably as high as possible, but it is not preferable to add a large amount of the high specific gravity filler to the cover composition, because the high specific gravity filler is generally a colored material.

The slab hardness and the density of the intermediate layer composition is appropriately adjusted by selecting the combination of the resin components, and controlling the amount of the additives.

The intermediate layer is formed, for example, by covering the center with the intermediate layer composition. An embodiment for molding the intermediate layer is not particularly limited, and includes an embodiment which comprises injection molding the intermediate layer composition directly onto the core, or an embodiment which comprises molding the intermediate layer composition into a half hollow-shell, covering the core with the two hollow-shells and subjecting the core with the two hollow shells to the compression-molding for 1 to 5 minutes at the temperature of 130°C. to 170°C.

The thickness of the intermediate layer is preferably 0.5 mm or more, preferably 0.6 mm or more, and is preferably 1.2 mm or less, more preferably 1.0 mm or less, and even more preferably 0.9 mm or less. If the thickness of the intermediate layer is 1.2 mm or less, since the core becomes relatively large, the repulsion of the golf ball is enhanced, while if the thickness of the intermediate layer is 0.5 mm or more, since

the inertia moment becomes high due to the large effect of the intermediate layer having the high specific gravity, the even lower spin is obtained.

In the above preferable embodiment, the cover composition preferably has a slab hardness of 57 or more, more preferably 59 or more, even more preferably 61 or more in Shore D hardness. If the cover composition has a slab hardness of 57 or more, the effect of the low spin on the driver shot becomes large, resulting in the greater flight distance. The cover composition preferably has a slab hardness of 66 or less in Shore D hardness. If the cover composition has a slab hardness of 66 or less, the shot feeling is more enhanced. Herein, the slab hardness of the cover composition is a measured hardness of the cover composition that is molded into a sheet form by a measuring method described later.

In the present invention, the thickness of the cover of the golf ball is preferably 0.3 mm or more, more preferably 0.4 mm or more, even more preferably 0.5 mm or more, and is preferably 1.0 mm or less, more preferably 0.9 mm or less, even more preferably 0.8 mm or less. If the cover has a thickness of 0.3 mm or more, it is easy to mold the cover and the workability is improved. On the other hand, if the cover has a thickness of 1.0 mm or less, since the intermediate layer having the high specific gravity can be disposed in the relatively outer part of the golf ball, the effect of the low spin on the driver shot becomes large due to the outer heavy inner right structure. Herein, the thickness is measured at the portion where the dimples are not formed, that is the thickness under the land 12 (refer to FIG. 1), and the thicknesses measured at least 4 portions are averaged.

When the golf ball of the present invention has a diameter in a range from 40 mm to 45 mm, a compression deformation amount of the golf ball (an amount of compression of the golf ball in the compression direction thereof) when applying an initial load of 98 N to a final load of 1275 N to the golf ball is preferably 2.5 mm or more, more preferably 2.7 mm or more, even more preferably 3.0 mm or more, and is preferably 4.0 mm or less, more preferably 3.7 mm or less, even more preferably 3.5 mm or less. By causing the compression deformation amount to be 2.5 mm or more, the desirable shot feeling is obtained. By causing the compression deformation amount to be 4.0 mm or less, the good repulsion is obtained.

The golf ball of the present invention is not particularly limited on the structure thereof, as long as it comprise a core consisting of at least one layer and an intermediate layer covering the core and a cover covering the intermediate layer. As the structure of the golf ball of the present invention, it may be a three-piece golf ball having a single-layered core and an intermediate layer covering the single-layered core, and a cover covering the intermediate layer; a four-piece golf ball comprising a core consisting of a center and a surrounding layer covering the center, an intermediate layer covering the core, and the cover covering the intermediate layer; a multi-piece golf ball having a multi-piece core consisting of a center and multi-piece or multi-layer of surrounding layers covering the center, an intermediate layer covering the multi-piece core, and a cover covering the intermediate layer. Among them, the present invention can be preferably applied to the three-piece golf ball having a single-layered core and an intermediate layer covering the single-layered core, and a cover covering the intermediate layer.

The present invention may further include a coated golf ball that comprises a golf ball body and a paint film covering the golf ball body, wherein the golf ball body comprises a core consisting of at least one layer, an intermediate layer covering the core and a cover covering the intermediate layer.

## EXAMPLES

10 Hereinafter, the present invention will be described in detail by way of example. The present invention is not limited to examples described below. Various changes and modifications can be made without departing from the spirit and scope of the present invention.

### (1) Hardness of Core and Golf ball (Shore D Hardness)

A type P1 or type LA1 auto loading durometer manufactured by Kobunshi Keiki Co., Ltd., provided with a Shore D type spring hardness tester prescribed in ASTM-D2240 was used to measure the surface hardness and the center hardness 20 of the core and the golf ball. Shore D hardness measured at the surfaces of the core and the golf ball are defined as the surface hardness of the core, and the golf ball, respectively. The core was cut into two hemispheres to obtain a cut plane, and a Shore D hardness measured at the center of the cut plane was 25 used as the center hardness of the core.

### (2) Compression Deformation Amount (mm)

A compression deformation amount of the golf ball or the core (a shrinking amount of the golf ball or the core in the compression direction thereof), when applying a load from 98 30 N as an initial load to 1275 N as a final load to the golf ball or the core, was measured.

### (3) Melt Viscosity Measure by a Flow Tester

The melt viscosity of a pellet-form sample was measured 35 under the following conditions by using a flow characteristics evaluation apparatus (Flow Tester CFT-500D, manufactured by Shimadzu Corporation).

#### Measuring Conditions

40 Die length: 1 mm

Die diameter: 1 mm

Load: 294 N

Temperature: 190° C.

### (4) Melt Viscosity (Pa·s) Measured by a Brookfield Viscometer

The melt viscosity of (b) the low melt viscosity ionomer resin heated at the temperature of 190° C. was measured by a brookfield viscometer (BL type viscometer available from Tokyo Keiki Inc.). Rotor No. 4 was used at a rotation speed of 50 6 rpm.

### (5) Content of Divalent Metal (Mole)

The content of the divalent metal was determined using ICP atomic emission spectrometer (Hitachi, Ltd. "P-410"). Specifically, 6 ml of concentrated sulfuric acid was added to 55 100 mg of the cover composition, and the mixture was subjected to the extraction (acid decomposition) with a microwave decomposition equipment (Microstone, ETHOS). To the extracted solution, water was added to prepare 250 ml of measurement sample for ICP analysis. From the obtained results, the content of the divalent metal per 100 g of the resin component of the cover composition was calculated according to the following mathematical expression.

$$\text{Divalent metal content (mole)} = \frac{[\text{mass (g) of the divalent metal per 100 g of the resin component contained in the cover composition}]}{[\text{atomic weight (g/mole) of each divalent metal}]} \quad [\text{Mathematical Expression}]$$

## (6) Melt Flow Rate (MFR) (g/10 min)

The MFR was measured using a flow tester (Shimadzu flow tester CFT-100C manufactured by Shimadzu Corporation) in accordance with JIS K7210. The measurement was conducted under the conditions of the measurement temperature 190° C. and the load of 2.16 kg.

## (7) Slab Hardness (Shore D Hardness)

Sheets with a thickness of about 2 mm were produced by injection molding the cover composition and the intermediate layer composition, and stored at 23° C. for two weeks. Three or more of these sheets were stacked on one another so as not to be affected by the measuring substrate on which the sheets were placed, and the stack was measured with a type P1 or type LA1 auto loading durometer manufactured by Kobunshi Keiki Co., Ltd., provided with a Shore D type spring hardness tester prescribed in ASTM-D2240.

## (8) Bending Stiffness (MPa)

A sheet with a thickness of about 2 mm was produced by injection molding the cover composition, and stored at 23° C. for two weeks. The bending stiffness was measured according to JIS K7106. The measurement was conducted under the conditions of the temperature 23° C. and humidity 50RH %.

## (9) Repulsion Resilience

A sheet with a thickness of about 2 mm was produced by a hot press molding from the cover composition. A circle-shaped test piece having a diameter of 28 mm was cut out of this sheet, and 6 pieces of the test piece were stacked to prepare a cylindrical test piece having a thickness of about 12 mm and a diameter of 28 mm. The cylindrical test piece was subjected to the Lupke type repulsion resilience test (testing temperature 23° C., humidity 50RH %). Preparation of the test piece and the testing method are based on JIS K6255.

## (10) Adhesion of Paint Film (Durability of Paint Film)

Each painted golf ball was hit 100 times repeatedly with a driver attached to a swing robot manufactured by TRUETEMPER CO, at the head speed of 45 m/sec. The degree of the peeling off of the paint film was observed and evaluated based on the following criteria.

E(Excellent): The paint film did not peel off at all.

G(Good): The area where the paint film peeled off was less than 1 mm<sup>2</sup>.

F(Fair): The area where the paint film peeled off was from 1 mm<sup>2</sup> to 4 mm<sup>2</sup>.

P(Poor): The area where the paint film peeled off was more than 4 mm<sup>2</sup>.

## (11) Coefficient of Repulsion

A 198.4 g of metal cylindrical object was forced to collide with each golf ball at a speed of 40 m/sec, and the speeds of the cylindrical object and the golf ball before and after the collision were measured. Based on these speeds and the mass of each object, coefficient of repulsion for each golf ball was calculated. The measurement was conducted by using twelve of each golf ball, and the average value was regarded as the coefficient of repulsion for the golf ball. For golf balls No. 1 to No. 17, the coefficient of repulsion of golf ball No. 11 was defined as an index of 100.0, and the coefficient of repulsion of each golf ball was represented by converting the coefficient of repulsion of each golf ball into this index. For golf balls No. 18 to No. 42, the coefficient of repulsion of golf ball No. 39 was defined as an index of 100.0, and the coefficient of repulsion of each golf ball was represented by converting the coefficient of repulsion of each golf ball into this index.

## (12) Durability

A metal-headed W#1 driver was installed on a swing robot M/C manufactured by Golf Laboratories, Inc. Each golf ball was hit at a head speed of 45 m/sec. This procedure was repeated, and the number of hits required to break the golf ball was counted. The number of hits for golf ball No. 11 was defined as an index of 100, and the durability of each golf ball was represented by converting the number of hits for each golf ball into this index. A greater index value indicates that the durability of the golf ball is excellent.

## (13) Low Temperature Durability A (Golf Balls No. 1 to No. 17)

Ten golf balls for each golf ball were made to collide with a metal board with an air gun at the speed of 45 m/sec., immediately after stored at the temperature of -10° C. for 1 day. This procedure was repeated, and the number of hits required to break the golf ball was counted. The results of the ten golf balls were averaged. The results were shown by the actual number of collision times. In the case that the golf ball was not broken even at the 50 times collision, "NB (not broken)" was shown.

## (14) Low Temperature Durability B (Golf Balls No. 18 to No. 42)

A metal-head driver was installed on a swing robot manufactured by TRUETEMPER CO, and the head speed was set to 45 m/sec. Each golf ball was stored in a constant temperature reservoir kept at the temperature of -10° C. for 24 hours, and then hit with a driver at the speed of 45 m/sec. to collide with a metal board. This procedure was repeated, and the number of hits required to break the golf ball was counted. It is noted that there was a case where the golf ball looks unbroken but a crack occurs in the intermediate layer. In such a case, whether or not the golf ball was broken was determined based on deformation of the golf ball and difference in sound at hitting of the golf ball. The number of hits for golf ball No. 39 was defined as an index of 100, and the low-temperature durability of each golf ball was represented by converting the number of hits for each golf ball into this index. A greater index value indicates that the durability of the golf ball is excellent.

## (15) Shot Feeling (Golf Balls No. 18 to No. 42)

An actual hitting test was carried out by ten amateur golfers (high skill) using a driver (#W1 driver), and the shot feeling was evaluated according to the following four criteria.

E(Excellent): Extremely soft feeling.

G(Good): Relatively soft feeling.

F(Fair): Relatively hard feeling.

P(Poor): Hard feeling.

## (16) Density of the Intermediate Layer (Golf Balls No. 18 to No. 42)

The intermediate layer composition was formed into a pellet, and the density of the pellet was measured in a solvent of ethanol with ARCHIMEDES available from Chyo balance Corporation.

## (17) Flight Distance (Golf Balls No. 18 to No. 42)

A metal-headed W#1 driver (XXIO S, loft: 10°, manufactured by SR1Sports Limited) was installed on a swing robot M/C manufactured by TRUETEMPER CO. Golf balls were hit at a head speed of 45 m/sec, and the flight distances (the distance from the launch point to the stop point) were measured. This measurement was conducted ten times for each golf ball, and the average value was used as the measurement value for the golf ball.

## (18) Direction Stability (Golf Balls No. 18 to No. 42)

A metal-headed W#1 driver (XXIO S, loft: 10°, manufactured by SRI Sports Limited) was installed on a swing robot M/C manufactured by TRUETEMPER CO so that the club face is in a direction orthogonal to the hitting direction. Then, golf balls were hit with a driver having club face open by 2° and close by 2° to the hitting direction, respectively. The distances between the stop point hit with a driver having a club face open by 2° and the stop point hit with a driver having a club face close by 2° were measured. The parallel lines to the hitting direction were drawn to pass through the respective two stop points, and the distance between the parallel lines were measured. This measurement was conducted ten times for each golf ball, and the average value was used as the measurement value for the golf ball.

[Production of Golf Balls No. 1 to No. 17]

## (1) Production of Core

The core rubber compositions having the formulations shown in Table 1 were kneaded and heat-pressed in upper and lower molds, each having a hemispherical cavity, at 170° C. for 15 minutes to prepare spherical cores having a diameter of 41.2 mm. The amount of barium sulfate was adjusted appropriately to make a golf ball have a weight of 45.4 g.

rpm, and screw L/D=35, and the mixtures were heated to 160 to 230° C. at the die position of the extruder.

## (3) Production of Golf Ball Body

Golf balls were produced by injection-molding the cover composition onto the spherical core to form a cover. Upper and lower molds have a spherical cavity with pimples, a part of which serves as a hold pin which is extendable and retractable. The hold pins were protruded to hold the core, the resin 5 heated to 210° C. was charged into the mold under a pressure of 80 tons within 0.3 seconds, and cooled for 30 seconds. Then, the mold was opened, and the golf ball body was taken out from the mold. The surface of the obtained golf ball body 10 were treated with sandblast, marked, and painted with a clear paint. As a clear paint, the following paint was used. The paint was dried in an oven at 40° C. to form a paint film having a thickness of 10 µm, and golf balls having a diameter of 42.8 mm and a mass of 45.4 g were obtained. The evaluation 15 results of the obtained golf ball are shown in Tables 2 to 5.

[Preparation of Clear Paint]

## (i) Base Material: Urethane Polyol

60 parts by mass of PTMG250 (BASF Co., polyoxytetramethylene glycol having a molecular weight of 250), 54 parts by

TABLE 1

|             |                                     | Core No.             |                      |                      |                      |
|-------------|-------------------------------------|----------------------|----------------------|----------------------|----------------------|
|             |                                     | A                    | B                    | C                    | D                    |
| Formulation | Polybutadiene                       | 100                  | 100                  | 100                  | 100                  |
|             | Zinc acrylate                       | 34                   | 34                   | 34                   | 34                   |
|             | Zinc oxide                          | 5                    | 5                    | 5                    | 5                    |
|             | Diphenyl disulfide                  | 0.5                  | 0.5                  | 0.5                  | 0.5                  |
|             | Dicumyl peroxide                    | 0.8                  | 0.8                  | 0.8                  | 0.8                  |
|             | Barium sulfate                      | Appropriate Amount*) | Appropriate Amount*) | Appropriate Amount*) | Appropriate Amount*) |
| Properties  | Diameter (mm)                       | 41.2                 | 38.2                 | 40.4                 | 41.8                 |
|             | Compression deformation amount (mm) | 3.2                  | 3.2                  | 3.2                  | 3.2                  |
|             | Center hardness (Shore D)           | 40                   | 40                   | 40                   | 40                   |
|             | Surface hardness (Shore D)          | 53                   | 53                   | 53                   | 53                   |
|             |                                     |                      |                      |                      |                      |

Formulation: parts by mass

\*)Depending on the cover composition, adjustment was made such that the golf ball had a mass of 45.4 g.

Polybutadiene rubber: "BR-730 (high-cis polybutadiene)" manufactured by JSR Corporation.

Zinc acrylate: "ZNDA-90S" manufactured by Nihon Jyoryu Kogyo Co., Ltd.

Zinc oxide: "Ginrei R" manufactured by Toho Zinc Co., Ltd.

Barium sulfate: "Barium Sulfate BD" manufactured by Sakai Chemical Industry Co., Ltd.

Diphenyl disulfide: manufactured by Sumitomo Seika Chemicals Co., Ltd.

Dicumyl peroxide: "Percumyl (registered trademark) D" manufactured by NOF Corporation.

## (2) Preparation of Cover Composition

Blending materials shown in Tables 2 to 5 were mixed with a twin-screw kneading extruder to prepare cover compositions in the pellet form. The extruding conditions were a screw diameter of 45 mm, a screw rotational speed of 200

mass of 550U (Sumitomo-Bayer Urethane Co., Ltd, branched polyol having a molecular weight of 550) were dissolved into 120 parts by mass of the solvent (toluene and methylethylketone). The dibutyl-tin-dilaurylate was added in an amount of 55 0.1 mass % with respect to the total base material. While keeping this polyol at the temperature of 80° C., 66 parts by mass of isophorone diisocyanate was slow-added into the polyol to obtain a urethane polyol having a solid content of 60 mass %, hydroxyl value of 75 mg KOH/g, and a weight average molecular weight of 7808.

(ii) Curing agent: Isophorone diisocyanate available from Sumitomo-Bayer Urethane Co., LTD.

(iii) Mixing ratio: NCO (curing agent)/OH (base material)=1.2 molar ratio.

TABLE 2

|                      |                                                         | Golf ball No. |       |       |       |       |
|----------------------|---------------------------------------------------------|---------------|-------|-------|-------|-------|
|                      |                                                         | 1             | 2     | 3     | 4     | 5     |
| Cover composition    | Core No.                                                | A             | B     | C     | D     | A     |
| Resin component      | (a) Himilan 1555 (Na)                                   | 30            | 30    | 30    | 30    | 30    |
|                      | component Himilan AM7329 (Zn)                           | 30            | 30    | 30    | 30    | 30    |
|                      | (b) Aclyn201 (Ca)                                       | —             | —     | —     | —     | 40    |
|                      | component Aclyn295 (Zn)                                 | 40            | 40    | 40    | 40    | —     |
|                      | AC 540                                                  | —             | —     | —     | —     | —     |
| Polyethylene         | Hi-wax 100P                                             | —             | —     | —     | —     | —     |
| Fatty acid           | Behenic acid                                            | —             | —     | —     | —     | —     |
|                      | Stearic acid                                            | —             | —     | —     | —     | —     |
|                      | (c) Nucrel 1050H                                        | —             | —     | —     | —     | —     |
|                      | component Nucrel 2050H                                  | —             | —     | —     | —     | —     |
| Titanium oxide       |                                                         | 4             | 4     | 4     | 4     | 4     |
| Material Properties  | Divalent metal content (mole per 100 g resin component) | 0.027         | 0.027 | 0.027 | 0.027 | 0.041 |
|                      | Melt flow rate (g/10 min)                               | 45            | 45    | 45    | 45    | 40    |
|                      | Slab hardness (Shore D)                                 | 59            | 59    | 59    | 59    | 59    |
|                      | Bending stiffness (MPa)                                 | 120           | 120   | 120   | 120   | 125   |
|                      | Repulsion resilience (%)                                | 48            | 48    | 48    | 48    | 49    |
| Golf ball evaluation | Cover thickness (mm)                                    | 0.8           | 2.3   | 1.2   | 0.5   | 0.8   |
|                      | Cover hardness (Shore D)                                | 63            | 63    | 63    | 63    | 63    |
|                      | Compression deformation amount (mm)                     | 3.04          | 2.40  | 2.90  | 3.10  | 3.04  |
|                      | Repulsion property (Index)                              | 100.2         | 100.6 | 100.3 | 100.2 | 100.1 |
|                      | Paint adhesion                                          | G             | G     | G     | G     | G     |
|                      | Durability (Index)                                      | 150           | 230   | 180   | 120   | 145   |
|                      | Low-temperature Durability (Times)                      | NB            | NB    | NB    | NB    | NB    |

Formulation: parts by mass,

NB: Not broken

TABLE 3

|                      |                                                         | Golf ball No. |       |       |       |       |
|----------------------|---------------------------------------------------------|---------------|-------|-------|-------|-------|
|                      |                                                         | 6             | 7     | 8     | 9     | 10    |
| Cover composition    | Core No.                                                | A             | C     | A     | A     | A     |
| Resin component      | (a) Himilan 1555 (Na)                                   | —             | 40    | —     | —     | —     |
|                      | component Himilan AM7329 (Zn)                           | 70            | 40    | 65    | 65    | 65    |
|                      | (b) Aclyn201 (Ca)                                       | 30            | —     | —     | —     | —     |
|                      | component Aclyn295 (Zn)                                 | —             | 20    | 10    | 10    | 20    |
|                      | AC 540                                                  | —             | —     | —     | —     | —     |
| Polyethylene         | Hi-wax 100P                                             | —             | —     | —     | —     | —     |
| Fatty acid           | Behenic acid                                            | —             | —     | —     | —     | —     |
|                      | Stearic acid                                            | —             | —     | —     | —     | —     |
|                      | (c) Nucrel 1050H                                        | —             | —     | 25    | —     | 15    |
|                      | component Nucrel 2050H                                  | —             | —     | —     | 25    | —     |
| Titanium oxide       |                                                         | 4             | 4     | 4     | 4     | 4     |
| Material Properties  | Divalent metal content (mole per 100 g resin component) | 0.051         | 0.025 | 0.032 | 0.032 | 0.035 |
|                      | Melt flow rate (g/10 min)                               | 25            | 10    | 33    | 32    | 23    |
|                      | Slab hardness (Shore D)                                 | 59            | 60    | 57    | 59    | 59    |
|                      | Bending stiffness (MPa)                                 | 204           | 240   | 173   | 197   | 220   |
|                      | Repulsion resilience (%)                                | 49            | 53    | 45    | 45    | 46    |
| Golf ball Evaluation | Cover thickness (mm)                                    | 0.8           | 1.2   | 0.8   | 0.8   | 0.8   |
|                      | Cover hardness (Shore D)                                | 64            | 65    | 61    | 64    | 64    |
|                      | Compression deformation amount (mm)                     | 3.01          | 2.86  | 3.02  | 3.01  | 2.99  |
|                      | Repulsion property (Index)                              | 100.1         | 100.4 | 100.1 | 100.2 | 100.2 |
|                      | Paint adhesion                                          | G             | G     | G     | G     | G     |
|                      | Durability (Index)                                      | 170           | 170   | 140   | 150   | 150   |
|                      | Low-temperature Durability (Times)                      | NB            | NB    | NB    | NB    | NB    |

Formulation: parts by mass,

NB: Not broken

TABLE 4

|                      |                     | Core No.      | Golf ball No.                               |             |             |             |             |
|----------------------|---------------------|---------------|---------------------------------------------|-------------|-------------|-------------|-------------|
|                      |                     |               | 11                                          | 12          | 13          | 14          | 15          |
| Cover composition    | Resin component     | (a) component | Himilan 1555 (Na)<br>Himilan AM7329 (Zn)    | 41<br>45    | 41<br>45    | 40<br>45    | 45<br>50    |
|                      |                     | (b) component | Aclyn201 (Ca)<br>Aclyn295 (Zn)              | —<br>—      | —<br>—      | —<br>—      | —<br>—      |
|                      |                     | (c) component | AC 540<br>Polyethylene<br>Fatty acid        | —<br>—<br>6 | —<br>—<br>6 | —<br>—<br>5 | —<br>—<br>— |
|                      |                     |               | Hi-wax 100P<br>Behenic acid<br>Stearic acid | —<br>—<br>— | —<br>—<br>5 | —<br>—<br>— | 5           |
|                      |                     |               | Nucrel 1050H<br>Nucrel 2050H                | 8<br>—      | 8<br>—      | 10<br>—     | —<br>—      |
|                      | Titanium oxide      |               | Divalent metal content (mole)               | 4           | 4           | 4           | 4           |
|                      | Material Properties |               | per 100 g resin component                   | 0.020       | 0.020       | 0.020       | 0.022       |
|                      |                     |               | Melt flow rate (g/10 min)                   | 33          | 33          | 33          | 28          |
|                      |                     |               | Slab hardness (Shore D)                     | 59          | 59          | 59          | 62          |
|                      |                     |               | Bending stiffness (MPa)                     | 168         | 168         | 162         | 171         |
|                      |                     |               | Repulsion resilience (%)                    | 40          | 40          | 41          | 43          |
| Golf ball Evaluation |                     |               | Cover thickness (mm)                        | 0.8         | 0.5         | 0.8         | 0.8         |
|                      |                     |               | Cover hardness (Shore D)                    | 63          | NG*)        | 63          | 66          |
|                      |                     |               | Compression deformation amount (mm)         | 3.02        |             | 3.02        | 2.98        |
|                      |                     |               | Repulsion property (Index)                  | 100.0       |             | 100.0       | 100.0       |
|                      |                     |               | Paint adhesion                              | P           |             | P           | P           |
|                      |                     |               | Durability (Index)                          | 100         |             | 98          | 105         |
|                      |                     |               | Low-temperature Durability (Times)          | 3           |             | 3           | 10          |
|                      |                     |               |                                             |             |             |             | 7           |

Formulation: parts by mass,

NB: Not broken,

NG: Impossible to mold.

TABLE 5

|                      |                     | Core No.      | Golf ball No.                               |                  |
|----------------------|---------------------|---------------|---------------------------------------------|------------------|
|                      |                     |               | 16                                          | 17               |
| Cover composition    | Resin component     | (a) component | Himilan 1555 (Na)<br>Himilan AM7329 (Zn)    | 50<br>50         |
|                      |                     | (b) component | Aclyn201 (Ca)<br>Aclyn295 (Zn)              | —<br>—<br>50     |
|                      |                     | (c) component | AC 540<br>Polyethylene<br>Fatty acid        | —<br>—<br>—<br>— |
|                      |                     |               | Hi-wax 100P<br>Behenic acid<br>Stearic acid | —<br>—<br>—<br>— |
|                      |                     |               | Nucrel 1050H<br>Nucrel 2050H                | —<br>—           |
|                      | Titanium oxide      |               | Divalent metal content (mole)               | 4                |
|                      | Material Properties |               | per 100 g resin component                   | 0.022            |
|                      |                     |               | Melt flow rate (g/10 min)                   | 8                |
|                      |                     |               | Slab hardness (Shore D)                     | 63               |
|                      |                     |               | Bending stiffness (MPa)                     | 264              |
|                      |                     |               | Repulsion resilience (%)                    | 55               |
| Golf ball evaluation |                     |               | Cover thickness (mm)                        | 0.8              |
|                      |                     |               | Cover hardness (Shore D)                    | NG*)             |
|                      |                     |               | Compression deformation amount (mm)         | 3.02             |
|                      |                     |               | Repulsion property (Index)                  | 98.9             |
|                      |                     |               | Paint adhesion                              | P                |
|                      |                     |               | Durability (Index)                          | 85               |
|                      |                     |               | Low-temperature Durability (Times)          | 1                |

Formulation: parts by mass,

NG: Impossible to mold

Notes on tables 2 to 5

Formulation: parts by mass

Himilan 1555: Sodium ion neutralized ethylene-methacrylic acid copolymer ionomer resin (Melt viscosity (190° C.) measured by a flow tester: 540 Pa·s, melt flow rate (190° C.\*2.16 kg): 10 g/10 min) available from Du Pont-Mitsui Polymers Co., Ltd

Himilan AM7329: Zinc ion neutralized ethylene-methacrylic acid copolymer ionomer resin (Melt viscosity (190° C.) measured by a flow tester: 1,100 Pa·s, melt flow rate (190° C.\*2.16 kg): 5 g/10 min) available from Du Pont-Mitsui Polymers Co., Ltd

29

Mixture (mass ratio 1:1) of Himilan 1555 and Himilan AM7329: melt viscosity (190° C.) measured by a flow tester: 850 Pa·s.

AC540: Binary copolymer composed of ethylene and  $\alpha,\beta$ -unsaturated carboxylic acid having 3 to 8 carbon atoms (Brookfield melt viscosity (190° C.): 0.6 Pa·s) available from Honeywell

Aclyn201: Calcium neutralized binary copolymer composed of ethylene and  $\alpha,\beta$ -unsaturated carboxylic acid having 3 to 8 carbon atoms (Brookfield melt viscosity (190° C.): 5.5 Pa·s, melt flow rate (190° C.\*2.16 kg): 185 g/10 min) available from Honeywell

Aclyn295: Zinc neutralized binary copolymer composed of ethylene and  $\alpha,\beta$ -unsaturated carboxylic acid having 3 to 8 carbon atoms (Brookfield melt viscosity (190° C.): 4.5 Pa·s, melt flow rate (190° C.\*2.16 kg): 1,200 g/10 min) available from Honeywell

Hi-wax 100P: Hi density type polyethylene wax (Brookfield melt viscosity (190° C.): 0.02 Pa·s) available from Mitsui Chemicals, INC

Behenic acid: "NAA-222S powder" available from NOF Corporation

Stearic acid: "Powder Stearic acid TUBAKI" available from NOF Corporation

Nucrel 1050H: ethylene-methacrylic acid copolymer (melt viscosity (190° C.) measured by a flow tester: 6 Pa·s, melt flow rate (190° C.\*2.16 kg): 500 g/10 min) available from Du Pont-Mitsui Polymers Co., Ltd.

Nucrel 0050H: ethylene-methacrylic acid copolymer (melt viscosity (190° C.) measured by a flow tester: 8 Pa·s, melt flow rate (190° C.\*2.16 kg): 500 g/10 min) available from Du Pont-Mitsui Polymers Co., Ltd.

30

Golf balls No. 11 and 13 are the cases that the low molecular weight material like a fatty acid was used. Bleed out occurred on the surface of the golf ball body and the adhesion of the paint film was not good. Further, the low-temperature durability was remarkably lowered. Golf ball No. 12 is the case that the cover having a thickness of 0.5 mm is formed from the same cover composition as that of Golf ball No. 11. Due to the insufficient fluidity of the cover composition, it was impossible to mold the cover. Golf balls No. 14 and No. 15 are the cases that the cover composition contains a low melt viscosity resin other than (b) the low melt viscosity ionomer resin. The adhesion of the paint film and the low-temperature durability were lowered. Golf ball No. 16 is the case that the cover composition does not contain a component corresponding to (b) the low melt viscosity ionomer resin. The cover composition showed a poor fluidity and thus it was impossible to mold the cover. Golf ball No. 17 is the case that the content of a component corresponding to (b) the low melt viscosity ionomer resin was too high. Durability was remarkably lowered.

The present invention provides a golf ball excellent in the fluidity, adhesion of the paint film, and repulsion, and further provides a golf ball which is excellent in the durability and low-temperature durability.

[Production of Golf Balls No. 18 to No. 42]

(1) Production of Core

The core rubber compositions having the formulations shown in Table 6 were kneaded and heat-pressed in upper and lower molds, each having a hemispherical cavity, at 170° C. for 20 minutes to prepare spherical cores.

TABLE 6

| Formulation | Polybutadiene      | Core composition No. |     |     |     |     |     |      |     |
|-------------|--------------------|----------------------|-----|-----|-----|-----|-----|------|-----|
|             |                    | 1                    | 2   | 3   | 4   | 5   | 6   | 7    | 8   |
|             | Zinc acrylate      | 100                  | 100 | 100 | 100 | 100 | 100 | 100  | 100 |
|             | Zinc oxide         | 29                   | 29  | 29  | 29  | 28  | 28  | 27.5 | 30  |
|             | Barium sulfate     | 10                   | 10  | 10  | 10  | 10  | 10  | 10   | 10  |
|             | Diphenyl disulfide | 12.5                 | 6.1 | 5.0 | 3.8 | 6.2 | 5.9 | 8.5  | 4.6 |
|             | Dicumyl peroxide   | 0.5                  | 0.5 | 0.5 | 0.5 | 0.5 | 0.5 | 0.5  | 0.5 |
|             |                    | 0.7                  | 0.7 | 0.7 | 0.7 | 0.7 | 0.7 | 0.7  | 0.7 |

Formulation: parts by mass

\*) Depending on the cover composition, adjustment was made such that the golf ball had a mass of 45.4 g.

As apparent from tables 2 to 5, the cover compositions No. 1 to No. 10 of the present invention showed a high melt flow rate and an excellent fluidity, in spite of showing the high repulsion. Further, during molding, bleed out of the low molecular weight material like the fatty acid was not observed and thus the obtained golf ball showed a good paint adhesion. Further, the cover compositions No. 1 to No. 10 of the present invention provided golf balls that are excellent in the durability and low-temperature durability.

Polybutadiene rubber: "BR-730 (high-cis polybutadiene)" manufactured by JSR Corporation.

Zinc acrylate: "ZNDA-90S" manufactured by Nihon Jyoryu Kogyo Co., Ltd.

Zinc oxide: "Ginrei R" manufactured by Toho Zinc Co., Ltd.

Barium sulfate: "Barium Sulfate BD" manufactured by Sakai Chemical Industry Co., Ltd.

Diphenyl disulfide: manufactured by Sumitomo Seika Chemicals Co., Ltd.

31

Dicumyl peroxide: "Percumyl (registered trademark) D"  
manufactured by NOF Corporation.

## (2) Preparation of Intermediate Layer Composition and Cover Composition

Blending materials shown in Tables 7, 9 to 13 were mixed with a twin-screw kneading extruder to prepare intermediate layer compositions and cover compositions in the pellet form. The extruding conditions were a screw diameter of 45 mm, a screw rotational speed of 200 rpm, and screw L/D=35, and the mixtures were heated to 160 to 230° C. at the die position of the extruder.

32

### (3) Production of Golf Ball Body

The intermediate layer compositions obtained above were injection-molded onto the spherical cores to form the intermediate layers covering the cores. Subsequently, golf balls were produced by injection-molding the cover composition onto the intermediate layer to form a cover. Upper and lower molds have a spherical cavity with pimples, a part of which serves as a hold pin which is extendable and retractable. The hold pins were protruded to hold the core, the resin heated to 210° C. was charged into the mold under a pressure of 80 tons within 0.3 seconds, and cooled for 30 seconds. Then, the mold

TABLE 7

| Intermediate layer composition |                | A    | B    | C    | D    | E    | F    | G    | H    |
|--------------------------------|----------------|------|------|------|------|------|------|------|------|
| Formulation                    | Surlyn 8945    | 35   | 35   | 35   | 35   | 48   | 25   | 32   | 45   |
|                                | Himilan AM7329 | 35   | 35   | 35   | 35   | 30   | 25   | 30   | 40   |
|                                | Rabalon T3221C | 30   | 30   | 30   | 30   | 22   | 50   | 38   | 15   |
|                                | Tungsten       | —    | 20   | 32   | 43   | 32   | 32   | 32   | 32   |
| Slab hardness (Shore D)        |                | 47   | 47   | 47   | 47   | 53   | 32   | 40   | 57   |
| Density (g/cm <sup>3</sup> )   |                | 0.94 | 1.12 | 1.22 | 1.32 | 1.22 | 1.22 | 1.22 | 1.22 |

### Formulation: parts by mass

### Note on table 7:

Surlyn 8945: Sodium ion neutralized ethylene-methacrylic acid copolymer ionomer resin available from E.I. du Pont de Nemours and Company

Himilan AM7329: Zinc ion neutralized ethylene-methacrylic acid copolymer ionomer resin available from Du Pont-Mitsui Polymers Co., Ltd

Rabalon T3221C: Polystyrene elastomer available from Mitsubishi Chemical Corporation.

Tungsten: Tungsten powder C50G available from A.L.M.T. Corp.

30 was opened, and the golf ball body were taken out from the  
31 mold. The surface of the obtained golf ball body were treated  
32 with sandblast, marked, and painted with a clear paint. The  
33 paint was dried in an oven at 40° C. to form a paint film having  
34 a thickness of 10  $\mu\text{m}$ , and golf balls having a diameter of 42.8  
35 mm and a mass of 45.4 g were obtained. As a clear paint, the  
36 same paint as that of Golf balls No. 1 to 17 were used.

40 The dimple patterns shown in table 8 and FIG. 2 and FIG. 3 were formed on the surface of the golf ball. In table 8, “diameter” of the dimple is depicted by  $D_i$  in FIG. 1 and “depth” means a distance between the tangential line and the deepest portion  $D_e$ .  $P$  means Pole in FIG. 3.

TABLE 8

| Kinds | Number | Curvature        |               |                |                            |                  |        | Plan view | Front view |
|-------|--------|------------------|---------------|----------------|----------------------------|------------------|--------|-----------|------------|
|       |        | Diameter<br>(mm) | Depth<br>(mm) | radius<br>(mm) | Area<br>(mm <sup>2</sup> ) | Occupancy<br>(%) |        |           |            |
| A     | 70     | 4.65             | 0.1380        | 19.65          | 1188.2                     | 82.1             | FIG. 2 | FIG. 3    |            |
| B     | 88     | 4.45             | 0.1380        | 18.01          | 1368.0                     |                  |        |           |            |
| C     | 56     | 4.30             | 0.1380        | 16.82          | 812.8                      |                  |        |           |            |
| D     | 26     | 4.20             | 0.1380        | 16.05          | 360.0                      |                  |        |           |            |
| E     | 42     | 4.10             | 0.1380        | 15.30          | 554.2                      |                  |        |           |            |
| F     | 20     | 3.90             | 0.1380        | 13.85          | 238.8                      |                  |        |           |            |
| G     | 18     | 3.20             | 0.1380        | 9.34           | 144.7                      |                  |        |           |            |
| H     | 8      | 3.00             | 0.1380        | 8.22           | 56.5                       |                  |        |           |            |
| Total | 328    | —                | —             | —              | 4723.2                     |                  |        |           |            |

The results of evaluations of the golf balls were also shown in tables 9 to 13.

TABLE 9

|                               |                                                         | Golf ball No.     |                     |       |       |       |       |
|-------------------------------|---------------------------------------------------------|-------------------|---------------------|-------|-------|-------|-------|
|                               |                                                         |                   | 18                  | 19    | 20    | 21    | 22    |
| Core                          | Core composition No.                                    |                   | 1                   | 2     | 3     | 4     | 5     |
| Diameter                      | (mm)                                                    | 39.8              | 39.8                | 39.8  | 39.8  | 39.8  | 39.8  |
| Core center hardness Ho       | Shore D                                                 | 39                | 39                  | 39    | 39    | 39    | 39    |
| Core surface hardness Hs      | Shore D                                                 | 52                | 52                  | 52    | 52    | 52    | 51    |
| Hardness difference (Hs - Ho) | Shore D                                                 | 13                | 13                  | 13    | 13    | 13    | 13    |
| Intermediate layer            | Intermediate layer composition No.                      |                   | A                   | B     | C     | D     | E     |
|                               | Slab hardness Hm                                        | Shore D           | 47                  | 47    | 47    | 47    | 53    |
|                               | Density                                                 | g/cm <sup>3</sup> | 0.94                | 1.12  | 1.22  | 1.32  | 1.22  |
|                               | Thickness                                               | (mm)              | 0.8                 | 0.8   | 0.8   | 0.8   | 0.8   |
| Cover                         | Resin component                                         | (a)               | Himilan 1555(Na)    | —     | —     | —     | —     |
|                               |                                                         |                   | Himilan AM7329 (Zn) | 70    | 70    | 70    | 70    |
|                               | (b)                                                     |                   | Aclyn 295 (Zn)      | 30    | 30    | 30    | 30    |
|                               |                                                         |                   | Aclyn 201 (Ca)      | —     | —     | —     | —     |
|                               | (c)                                                     |                   | Nucrel 1050H        | —     | —     | —     | —     |
|                               | Fatty acid                                              |                   | Behenic acid        | —     | —     | —     | —     |
|                               | Titanium oxide                                          |                   |                     | 3     | 3     | 3     | 3     |
|                               | Ultramarine blue                                        |                   |                     | 0.04  | 0.04  | 0.04  | 0.04  |
| Material Properties           | Divalent metal content (mole) per 100 g resin component |                   | 0.041               | 0.041 | 0.041 | 0.041 | 0.041 |
|                               | Slab hardness (Shore D)                                 |                   | 60                  | 60    | 60    | 60    | 60    |
|                               | Melt flow rate (g/10 min)                               |                   | 28                  | 28    | 28    | 28    | 28    |
|                               | Thickness (mm)                                          |                   | 0.7                 | 0.7   | 0.7   | 0.7   | 0.7   |
| Golf ball evaluation          | Compression deformation amount (mm)                     |                   | 3.4                 | 3.4   | 3.4   | 3.4   | 3.4   |
|                               | Repulsion coefficient (Index)                           |                   | 100.5               | 100.5 | 100.5 | 100.5 | 100.8 |
|                               | Flight distance (m)                                     |                   | 230                 | 232   | 234   | 235   | 234   |
|                               | Direction stability (m)                                 |                   | 8.2                 | 4.5   | 3.4   | 3.0   | 3.6   |
|                               | Low-temperature Durability                              |                   | 150                 | 150   | 150   | 150   | 150   |
|                               | Adhesion of Paint film                                  |                   | E                   | E     | E     | E     | E     |
|                               | Shot feeling                                            |                   | E                   | E     | E     | E     | G     |

Formulation: parts by mass

TABLE 10

|                               |                                                         | Golf ball No.     |                     |       |       |       |       |
|-------------------------------|---------------------------------------------------------|-------------------|---------------------|-------|-------|-------|-------|
|                               |                                                         |                   | 23                  | 24    | 25    | 26    | 27    |
| Core                          | Core composition No.                                    |                   | 3                   | 3     | 3     | 3     | 3     |
| Diameter                      | (mm)                                                    | 39.8              | 39.8                | 39.8  | 39.8  | 39.8  | 39.8  |
| Core center hardness Ho       | Shore D                                                 | 39                | 39                  | 39    | 39    | 39    | 39    |
| Core surface hardness Hs      | Shore D                                                 | 52                | 52                  | 52    | 52    | 52    | 52    |
| Hardness difference (Hs - Ho) | Shore D                                                 | 13                | 13                  | 13    | 13    | 13    | 13    |
| Intermediate layer            | Intermediate layer composition No.                      |                   | G                   | C     | C     | C     | C     |
|                               | Slab hardness Hm                                        | Shore D           | 40                  | 47    | 47    | 47    | 47    |
|                               | Density                                                 | g/cm <sup>3</sup> | 1.22                | 1.22  | 1.22  | 1.22  | 1.22  |
|                               | Thickness                                               | (mm)              | 0.8                 | 0.8   | 0.8   | 0.8   | 0.8   |
| Cover                         | Resin component                                         | (a)               | Himilan 1555 (Na)   | —     | —     | 20    | —     |
|                               |                                                         |                   | Himilan AM7329 (Zn) | 70    | 96    | 56    | 50    |
|                               | (b)                                                     |                   | Aclyn 295 (Zn)      | 30    | 4     | 44    | 30    |
|                               |                                                         |                   | Aclyn 201 (Ca)      | —     | —     | —     | 30    |
|                               | (c)                                                     |                   | Nucrel 1050H        | —     | —     | —     | —     |
|                               | Fatty acid                                              |                   | Behenic acid        | —     | —     | —     | —     |
|                               | Titanium oxide                                          |                   |                     | 3     | 3     | 3     | 3     |
|                               | Ultramarine blue                                        |                   |                     | 0.04  | 0.04  | 0.04  | 0.04  |
| Material Properties           | Divalent metal content (mole) per 100 g resin component |                   | 0.041               | 0.043 | 0.040 | 0.042 | 0.051 |
|                               | Slab hardness (Shore D)                                 |                   | 60                  | 62    | 58    | 61    | 60    |
|                               | Melt flow rate (g/10 min)                               |                   | 28                  | 11    | 30    | 27    | 25    |
|                               | Thickness (mm)                                          |                   | 0.7                 | 0.7   | 0.7   | 0.7   | 0.7   |
| Golf ball Evaluation          | Compression deformation amount (mm)                     |                   | 3.5                 | 3.4   | 3.5   | 3.4   | 3.4   |
|                               | Repulsion coefficient (Index)                           |                   | 100.4               | 100.8 | 100.2 | 100.6 | 100.9 |
|                               | Flight distance (m)                                     |                   | 233                 | 235   | 232   | 235   | 234   |
|                               | Direction stability (m)                                 |                   | 3.4                 | 3.5   | 4.0   | 3.5   | 3.6   |
|                               | Low-temperature Durability                              |                   | 160                 | 135   | 155   | 124   | 140   |
|                               | Adhesion of Paint film                                  |                   | E                   | E     | E     | E     | E     |
|                               | Shot feeling                                            |                   | E                   | E     | E     | E     | E     |

Formulation: parts by mass

TABLE 11

|                      |                                                         | Golf ball No. |                     |       |       |       |       |    |
|----------------------|---------------------------------------------------------|---------------|---------------------|-------|-------|-------|-------|----|
|                      |                                                         |               | 28                  | 29    | 30    | 31    | 32    |    |
| Core                 | Core composition No.                                    |               | 6                   | 8     | 3     | 3     | 3     |    |
|                      | Diameter (mm)                                           |               | 39.4                | 40.4  | 39.8  | 39.8  | 39.8  |    |
|                      | Core center hardness Ho                                 | Shore D       | 38                  | 40    | 39    | 39    | 39    |    |
|                      | Core surface hardness Hs                                | Shore D       | 51                  | 53    | 52    | 52    | 52    |    |
|                      | Hardness difference (Hs - Ho)                           | Shore D       | 13                  | 13    | 13    | 13    | 13    |    |
| Intermediate layer   | Intermediate layer composition No.                      |               | C                   | C     | C     | C     | C     |    |
|                      | Slab hardness Hm                                        | Shore D       | 47                  | 47    | 47    | 47    | 47    |    |
|                      | Density g/cm <sup>3</sup>                               |               | 1.22                | 1.22  | 1.22  | 1.22  | 1.22  |    |
|                      | Thickness (mm)                                          |               | 0.8                 | 0.8   | 0.8   | 0.8   | 0.8   |    |
|                      | Resin component                                         | (a)           | Himilan 1555 (Na)   | —     | —     | —     | —     |    |
| Cover                |                                                         | (b)           | Himilan AM7329 (Zn) | 70    | 70    | 60    | 74    | 46 |
|                      |                                                         | (c)           | Aclyn 295 (Zn)      | 30    | 30    | 20    | 20    | 20 |
|                      |                                                         |               | Aclyn 201 (Ca)      | —     | —     | —     | —     | —  |
|                      |                                                         |               | Nucrel 1050H        | —     | —     | 20    | 6     | 34 |
|                      | Fatty acid                                              |               | Behenic acid        | —     | —     | —     | —     | —  |
| Material Properties  | Titanium oxide                                          |               | 3                   | 3     | 3     | 3     | 3     |    |
|                      | Ultramarine blue                                        |               | 0.04                | 0.04  | 0.04  | 0.04  | 0.04  |    |
|                      | Divalent metal content (mole) per 100 g resin component |               | 0.041               | 0.041 | 0.033 | 0.039 | 0.027 |    |
|                      | Slab hardness (Shore D)                                 |               | 60                  | 60    | 58    | 60    | 57    |    |
|                      | Melt flow rate (g/10 min)                               |               | 28                  | 28    | 31    | 20    | 38    |    |
| Golf ball Evaluation | Thickness (mm)                                          |               | 0.9                 | 0.4   | 0.7   | 0.7   | 0.7   |    |
|                      | Compression deformation amount (mm)                     |               | 3.4                 | 3.4   | 3.5   | 3.4   | 3.5   |    |
|                      | Repulsion coefficient (Index)                           |               | 100.5               | 100.6 | 100.3 | 100.4 | 100.2 |    |
|                      | Flight distance (m)                                     |               | 233                 | 235   | 232   | 235   | 232   |    |
|                      | Direction stability (m)                                 |               | 4.9                 | 3.0   | 3.9   | 3.6   | 4.2   |    |
|                      | Low-temperature Durability                              |               | 155                 | 125   | 138   | 147   | 126   |    |
|                      | Adhesion of Paint film                                  |               | E                   | E     | E     | E     | E     |    |
|                      | Shot feeling                                            |               | G                   | E     | E     | E     | E     |    |

Formulation: parts by mass

TABLE 12

|                      |                                                         | Golf ball No. |                     |       |       |       |       |     |
|----------------------|---------------------------------------------------------|---------------|---------------------|-------|-------|-------|-------|-----|
|                      |                                                         |               | 33                  | 34    | 35    | 36    | 37    |     |
| Core                 | Core composition No.                                    |               | 3                   | 8     | 8     | 5     | 3     |     |
|                      | Diameter (mm)                                           |               | 39.8                | 39.8  | 39.8  | 39.8  | 39.8  |     |
|                      | Core center hardness Ho                                 | Shore D       | 39                  | 40    | 40    | 38    | 39    |     |
|                      | Core surface hardness Hs                                | Shore D       | 52                  | 53    | 53    | 51    | 52    |     |
|                      | Hardness difference (Hs - Ho)                           | Shore D       | 13                  | 13    | 13    | 13    | 13    |     |
| Intermediate layer   | Intermediate layer composition No.                      |               | C                   | C     | F     | H     | C     |     |
|                      | Slab hardness Hm                                        | Shore D       | 47                  | 47    | 32    | 57    | 47    |     |
|                      | Density g/cm <sup>3</sup>                               |               | 1.22                | 1.22  | 1.22  | 1.22  | 1.22  |     |
|                      | Thickness (mm)                                          |               | 0.8                 | 0.8   | 0.8   | 0.8   | 0.8   |     |
|                      | Resin component                                         | (a)           | Himilan 1555 (Na)   | —     | —     | —     | —     |     |
| Cover                |                                                         | (b)           | Himilan AM7329 (Zn) | 68    | 38    | 70    | 70    | 100 |
|                      |                                                         | (c)           | Aclyn 295 (Zn)      | 20    | 20    | 30    | 30    | —   |
|                      |                                                         |               | Aclyn 201 (Ca)      | —     | —     | —     | —     | —   |
|                      |                                                         |               | Nucrel 1050H        | 12    | 42    | —     | —     | —   |
|                      | Fatty acid                                              |               | Behenic acid        | —     | —     | —     | —     | —   |
| Material Properties  | Titanium oxide                                          |               | 3                   | 3     | 3     | 3     | 3     |     |
|                      | Ultramarine blue                                        |               | 0.04                | 0.04  | 0.04  | 0.04  | 0.04  |     |
|                      | Divalent metal content (mole) per 100 g resin component |               | 0.037               | 0.024 | 0.041 | 0.041 | 0.044 |     |
|                      | Slab hardness (Shore D)                                 |               | 59                  | 56    | 60    | 60    | 64    |     |
|                      | Melt flow rate (g/10 min)                               |               | 26                  | 44    | 28    | 28    | 5     |     |
| Golf ball Evaluation | Thickness (mm)                                          |               | 0.7                 | 0.7   | 0.7   | 0.7   | 0.7   |     |
|                      | Compression deformation amount (mm)                     |               | 3.4                 | 3.4   | 3.4   | 3.3   | NG*)  |     |
|                      | Repulsion coefficient (Index)                           |               | 100.3               | 100.1 | 99.8  | 100.6 |       |     |
|                      | Flight distance (m)                                     |               | 232                 | 228   | 228   | 235   |       |     |
|                      | Direction stability (m)                                 |               | 3.7                 | 4.4   | 3.3   | 3.7   |       |     |
|                      | Low-temperature Durability                              |               | 144                 | 101   | 160   | 145   |       |     |
|                      | Adhesion of Paint film                                  |               | E                   | E     | E     | E     |       |     |
|                      | Shot feeling                                            |               | E                   | E     | E     | E     | P     |     |

Formulation: parts by mass,  
NG: Impossible to mold

TABLE 13

|                      |                                       | Golf ball No.                                           |       |       |       |       |       |
|----------------------|---------------------------------------|---------------------------------------------------------|-------|-------|-------|-------|-------|
|                      |                                       |                                                         | 38    | 39    | 40    | 41    | 42    |
| Core                 | Core composition No.                  |                                                         | 3     | 3     | 3     | 7     | 8     |
|                      | Diameter (mm)                         | 39.8                                                    | 39.8  | 39.8  | 39.0  | 40.8  |       |
|                      | Core center hardness Ho Shore D       | 39                                                      | 39    | 39    | 37    | 40    |       |
|                      | Core surface hardness Hs Shore D      | 52                                                      | 52    | 52    | 50    | 53    |       |
|                      | Hardness difference (Hs - Ho) Shore D | 13                                                      | 13    | 13    | 13    | 13    |       |
| Intermediate layer   | Intermediate layer composition No.    | C                                                       | C     | C     | C     | C     |       |
|                      | Slab hardness Hm Shore D              | 47                                                      | 47    | 47    | 47    | 47    |       |
|                      | Density g/cm <sup>3</sup>             | 1.22                                                    | 1.22  | 1.22  | 1.22  | 1.22  |       |
|                      | Thickness (mm)                        | 0.8                                                     | 0.8   | 0.8   | 0.8   | 0.8   |       |
| Cover                | Resin component (a)                   | Himilan 1555 (Na)                                       | —     | —     | —     | —     | —     |
|                      |                                       | Himilan AM7329 (Zn)                                     | 50    | 70    | 85    | 70    | 70    |
|                      | (b)                                   | Aclyn 295 (Zn)                                          | 50    | —     | —     | 30    | 30    |
|                      |                                       | Aclyn 201 (Ca)                                          | —     | —     | —     | —     | —     |
|                      | (c)                                   | Nucrel 1050H                                            | —     | 30    | —     | —     | —     |
|                      | Fatty acid                            | Behenic acid                                            | —     | —     | 15    | —     | —     |
|                      | Titanium oxide                        |                                                         | 3     | 3     | 3     | 3     | 3     |
|                      | Ultramarine blue                      |                                                         | 0.04  | 0.04  | 0.04  | 0.04  | 0.04  |
| Material Properties  | Material Properties                   | Divalent metal content (mole) per 100 g resin component | 0.040 | 0.031 | 0.037 | 0.041 | 0.041 |
|                      | Slab hardness (Shore D)               | 56                                                      | 59    | 60    | 60    | 60    |       |
|                      | Melt flow rate (g/10 min)             | 35                                                      | 25    | 57    | 28    | 28    |       |
|                      | Thickness (mm)                        | 0.7                                                     | 0.7   | 0.7   | 1.1   | 0.2   |       |
| Golf ball Evaluation | Compression deformation amount (mm)   | 3.5                                                     | 3.4   | 3.4   | 3.4   | NG*)  |       |
|                      | Repulsion coefficient (Index)         | 99.8                                                    | 100.0 | 100.0 | 100.4 |       |       |
|                      | Flight distance (m)                   | 225                                                     | 234   | 234   | 229   |       |       |
|                      | Direction stability (m)               | 7.1                                                     | 3.7   | 3.8   | 7.2   |       |       |
|                      | Low-temperature Durability            | 160                                                     | 100   | 120   | 160   |       |       |
|                      | Adhesion of Paint film                | E                                                       | E     | P     | E     |       |       |
|                      | Shot feeling                          | E                                                       | E     | E     | F     |       |       |

Formulation: parts by mass,

NG: Impossible to mold

## Note on tables 9 to 13

Ultramarine blue: Ultramarine blue No1500 available from Daiichi Kogyo Company

Details of the other materials are described in Notes on tables 2 to 5.

Golf balls No. 18 to 29 are the cases that the cover is formed from the cover composition that contains, as a resin component, (a) the high melt viscosity ionomer resin and (b) the low melt viscosity ionomer resin in a specific amount as well as a divalent metal ion in an amount of at least 0.020 mole per 100 g of the resin component and that the cover thickness and the slab hardness of the intermediate layer composition fall within the range prescribed by the present invention. Golf balls No. 30 to 34 are the cases that the cover composition further contains (c) a nonionic thermoplastic resin in a specific amount. All of the cover composition used for these golf balls showed a high melt flow rate and an excellent fluidity, in spite of showing the high repulsion. Further, during molding, bleed out of the low molecular weight material like the fatty acid was not observed and thus the obtained golf ball showed a good paint adhesion. As a result, these golf balls were excellent in the repulsion coefficient, flight distance, low-temperature durability, adhesion of the paint film, and shot feeling.

Among them, golf balls No. 19 to 34 whose intermediate layer has a density of 1.10 g/cm<sup>3</sup> or more were excellent in direction stability. However, the shot feeling of golf ball No. 22 was slightly low because the intermediate layer composition has a slightly high slab hardness, and the shot feeling of golf ball No. 28 was also slightly low because the thickness of the cover is slightly thick. The workability in golf balls No. 24 and No. 31 were slightly low because the content of (a) component was high. Golf ball No. 34 was slightly inferior in flight distance due to the high content of (c) component.

Golf ball No. 35 is the case that intermediate layer composition has a slab hardness less than 35 in Shore D hardness. Repulsion coefficient was low and flight distance was not good. Golf ball No. 36 is the case that the intermediate layer composition has a slab hardness of 55 or more in shore D hardness. The shot feeling deteriorated.

Golf ball No. 37 is the case that the cover composition does not contain a component corresponding to (b) the low melt viscosity ionomer resin. The cover composition showed a poor fluidity and thus it was impossible to mold the cover having a thickness of 0.7 mm. Golf ball No. 38 is the case that the ratio (a) component to (b) component was small. The repulsion coefficient was low and the flight distance was not good. Golf ball No. 39 is the case that the cover composition does not contain (b) component but (c) component. The low-temperature durability was not improved due to the less amount of the divalent metal contained in the resin component, although the cover could be molded.

Golf ball No. 40 is the case that a fatty acid was used. Bleed out occurred on the surface of the golf ball body and the adhesion of the paint film was not good.

Golf ball No. 41 is the case that the cover has a thickness more than 1.0 mm, the shot feeling deteriorated. Further, because of the thick cover, the intermediate layer having a high density was disposed in a relatively inner part of the golf ball. Thus, the effect of the low spin on the driver shot was small and the flight distance and the direction stability were inferior. Golf ball No. 42 is the case that the cover having a thickness of 0.2 mm is formed from the same cover composition as that of golf ball No. 20. Due to the insufficient fluidity, the cover could not be molded.

The present invention provides a golf ball excellent in the adhesion of the paint film, low-temperature durability, flight distance and shot feeling on the shots as well as improves the

moldability of the cover. Further, the present invention provides a golf ball excellent in the direction stability on the shots.

This application is based on Japanese Patent applications No. 2008-237037 filed on Sep. 16, 2008, No. 2008-269361 filed on Oct. 20, 2008, and No. 2009-193330 filed on Aug. 24, 2009, the contents of which are hereby incorporated by reference.

The invention claimed is:

**1. A golf ball comprising:**

a core and a cover covering the core, wherein the cover is formed from a cover composition that contains as a resin component,

(a) a high melt viscosity ionomer resin having a melt viscosity (190° C.) ranging from 500 Pa·s to 100,000 Pa·s measured by a flow tester, and

(b) a low melt viscosity ionomer resin having a melt viscosity (190° C.) ranging from 1 Pa·s to 10 Pa·s measured by a Brookfield viscometer and a melt flow rate (190° C.

\*2.16 kg) ranging from 100 g/10 min to 2,000 g/10 min,

in a ratio of (a) the high melt viscosity ionomer resin/(b) the low melt viscosity ionomer resin being 55 mass % to 99 mass %/45 mass % to 1 mass %, wherein at least one of metal ions neutralizing carboxyl groups of (a) the high melt viscosity ionomer resin and/or (b) the low melt viscosity ionomer resin is a divalent metal ion and a content of the divalent metal ion per 100 g of the resin component is at least 0.020 mole, and wherein the cover composition has a melt flow rate (190° C. \*2.16 kg) ranging from 10 g/10 min to 100 g/10 min.

**2. The golf ball according to claim 1, wherein the content of the divalent metal ion per 100 g of the resin component is at least 0.030 mole.**

**3. The golf ball according to claim 1, wherein (a) the high melt viscosity ionomer resin contains one prepared by neutralizing at least a part of carboxyl groups in a binary copolymer composed of ethylene and a,  $\alpha$ , $\beta$ -unsaturated carboxylic acid having 3 to 8 carbon atoms with a metal ion, one prepared by neutralizing at least a part of carboxyl groups in a ternary copolymer composed of ethylene,  $\alpha$ , $\beta$ -unsaturated carboxylic acid having 3 to 8 carbon atoms, and  $\alpha$ , $\beta$ -unsaturated carboxylic acid ester with a metal ion, or a mixture thereof.**

**4. The golf ball according to claim 1, wherein (a) the high melt viscosity ionomer resin has a neutralization degree of carboxyl groups from 10 mole % to 90 mole % and (b) the low melt viscosity ionomer resin has a neutralization degree of carboxyl groups from 10 mole % to 100 mole %.**

**5. The golf ball according to claim 1, wherein the cover composition has a bending stiffness ranging from 100 MPa to 450 MPa and a repulsion resilience of 40% or more.**

**6. The golf ball according to claim 1, wherein the cover composition further comprises (c) a nonionic thermoplastic resin having a melt viscosity (190° C.) ranging from 5 Pa·s to 3,000 Pa·s measured by a flow tester, and contains each component in the content of (a) the high melt viscosity ionomer resin: 55 mass % to 70 mass %, (b) the low melt viscosity ionomer resin: 5 mass % to 20 mass %, and (c) the nonionic thermoplastic resin: 5 mass % to 40 mass %.**

**7. A golf ball comprising:**

a core and a cover covering the core,

wherein the cover is formed from a cover composition that contains as a resin component,

(a) a high melt viscosity ionomer resin having a melt viscosity (190° C.) ranging from 500 Pa·s to 100,000 Pa·s measured by a flow tester and consisting of one prepared by neutralizing at least a part of carboxyl groups in a binary copolymer composed of ethylene and  $\alpha$ , $\beta$ -unsat-

urated carboxylic acid having 3 to 8 carbon atoms with a metal ion, one prepared by neutralizing at least a part of carboxyl groups in a ternary copolymer composed of ethylene,  $\alpha$ , $\beta$ -unsaturated carboxylic acid having 3 to 8 carbon atoms and  $\alpha$ , $\beta$ -unsaturated carboxylic acid ester with a metal ion, or a mixture thereof, and

(b) a low melt viscosity ionomer resin having a melt viscosity (190° C.) ranging from 1 Pa·s to 10 Pa·s measured by a Brookfield viscometer and a melt flow rate (190° C.\*2.16 kg) ranging from 100 g/10min to 2,000 g/10min, and consisting of one prepared by neutralizing at least a part of carboxyl groups in a binary copolymer composed of ethylene and  $\alpha$ , $\beta$ -unsaturated carboxylic acid having 3 to 8 carbon atoms with a metal ion, one prepared by neutralizing at least a part of carboxyl groups in a ternary copolymer composed of ethylene,  $\alpha$ , $\beta$ -unsaturated carboxylic acid having 3 to 8 carbon atoms and  $\alpha$ , $\beta$ -unsaturated carboxylic acid ester with a metal ion, or a mixture thereof,

in a ratio of (a) the high melt viscosity ionomer resin/(b) the low melt viscosity ionomer resin being 55 mass % to 99 mass %/45 mass % to 1 mass %, wherein at least one of metal ions neutralizing carboxyl groups of (a) the high melt viscosity ionomer resin and/or (b) the low melt viscosity ionomer resin is a divalent metal ion and a content of the divalent metal ion per 100 g of the resin component is at least 0.020 mole, and wherein the cover composition has a melt flow rate (190° C.\*2.16 kg) ranging from 10 g/10 min to 100 g/10 min.

**8. The golf ball according to claim 7, wherein at least a part of carboxyl groups of (b) the low melt viscosity ionomer resin is neutralized with at least one metal ion selected from the group consisting of Na, Ca, Mg and Zn.**

**9. The golf ball according to claim 7, wherein at least a part of carboxyl groups of (a) the high melt viscosity ionomer resin is neutralized with at least one metal ion selected from the group consisting of Na, Ca, Mg and Zn.**

**10. The golf ball according to claim 7, wherein the cover composition further comprises (c) a nonionic thermoplastic resin having a melt viscosity (190° C.) ranging from 5 Pa·s to 3,000 Pa·s measured by a flow tester, and contains each component in the content of (a) the high melt viscosity ionomer resin: 55 mass % to 70 mass %, (b) the low melt viscosity ionomer resin: 5 mass % to 20 mass %, and (c) the nonionic thermoplastic resin: 10 mass % to 40 mass %.**

**11. The golf ball according to claim 10, wherein (c) the nonionic thermoplastic resin comprises a binary copolymer composed of ethylene and  $\alpha$ , $\beta$ -unsaturated carboxylic acid having 3 to 8 carbon atoms.**

**12. The golf ball according to claim 7, wherein the cover has a thickness ranging from 0.1 mm to 3 mm.**

**13. A golf ball comprising:**

a core consisting of at least one layer,

an intermediate layer covering the core, and

a cover covering the intermediate layer and having a thickness from 0.3 mm to 1.0 mm,

wherein the cover is formed from a cover composition that contains as a resin component,

(a) a high melt viscosity ionomer resin having a melt viscosity (190° C.) ranging from 500 Pa·s to 100,000 Pa·s measured by a flow tester and consisting of one prepared by neutralizing at least a part of carboxyl groups in a binary copolymer composed of ethylene and  $\alpha$ , $\beta$ -unsaturated carboxylic acid having 3 to 8 carbon atoms with a metal ion, one prepared by neutralizing at least a part of carboxyl groups in a ternary copolymer composed of ethylene,  $\alpha$ , $\beta$ -unsaturated carboxylic acid having 3 to 8

**41**

carbon atoms and  $\alpha,\beta$ -unsaturated carboxylic acid ester with a metal ion, or a mixture thereof, and  
 (b) a low melt viscosity ionomer resin having a melt viscosity (190° C.) ranging from 1 Pa·s to 10 Pa·s measured by a Brookfield viscometer and a melt flow rate (190° C.\*2.16 kg) ranging from 100 g/10 min to 2,000 g/10 min, and consisting of one prepared by neutralizing at least a part of carboxyl groups in a binary copolymer composed of ethylene and  $\alpha,\beta$ -unsaturated carboxylic acid having 3 to 8 carbon atoms with a metal ion, one prepared by neutralizing at least a part of carboxyl groups in a ternary copolymer composed of ethylene,  $\alpha,\beta$ -unsaturated carboxylic acid having 3 to 8 carbon atoms and  $\alpha,\beta$ -unsaturated carboxylic acid ester with a metal ion, or a mixture thereof,  
 in a ratio of (a) the high melt viscosity ionomer resin/(b) the low melt viscosity ionomer resin being 55 mass % to 99 mass %/45 mass % to 1 mass %, wherein at least one of the metal ions neutralizing carboxyl groups of (a) the high melt viscosity ionomer resin and/or (b) the low melt viscosity ionomer resin is a divalent metal ion and a content of the divalent metal ion per 100 g of the resin component is at least 0.020 mole,

**42**

wherein an intermediate layer composition forming the intermediate layer has a slab hardness from 35 to 55 in Shore D hardness, and wherein the cover composition has a melt flow rate (190° C.\*2.16 kg) ranging from 10 g/10 min to 100 g/10 min.

14. The golf ball according to claim 13, wherein the cover composition further comprises (c) a nonionic thermoplastic resin having a melt viscosity (190° C.) ranging from 5 Pa·s to 3,000 Pa·s measured by a flow tester, and contains each component in the content of (a) the high melt viscosity ionomer resin: 45 mass % to 70 mass %, (b) the low melt viscosity ionomer resin: 5 mass % to 25 mass %, and (c) the nonionic thermoplastic resin: 10 mass % to 40 mass %.

15. The golf ball according to claim 13, wherein the intermediate layer has a density of at least 1.10 g/cm<sup>3</sup>.

16. The golf ball according to claim 13, wherein the cover composition has a slab hardness of 57 or more in Shore D hardness.

20 17. The golf ball according to claim 13, wherein the core has a diameter of 39.1 mm or more.

\* \* \* \* \*